

Jan. 6, 1959

R. I. JAFFEE ET AL

2,867,534

TITANIUM BASE ALPHA DISPERSOID ALLOYS

Filed Jan. 23, 1957

3 Sheets-Sheet 1

FIG. 1.

EFFECT OF TEMPERING ON THE HARDNESS  
OF END-QUENCHED  $Ti-10Sn-7Cu$



INVENTORS  
ROBERT I. JAFFEE.  
HORACE R. OGDEN.  
BY

Ward, Neal, Haselton, Dime & McElhanon  
ATTORNEYS.

Jan. 6, 1959

R. I. JAFFEE ET AL

2,867,534

TITANIUM BASE ALPHA DISPERSOID ALLOYS

Filed Jan. 23, 1957

3 Sheets-Sheet 2

FIG. 2.

EFFECT OF INCREASING TIN CONTENT  
ON THE HARDNESS OF Ti-7Cu-BASE ALLOY



INVENTORS.  
ROBERT I. JAFFEE  
HORACE R. OGDEN.  
BY

Arard, Heath, Haselton, Orme & McElhanon  
ATTORNEYS.

Jan. 6, 1959

R. I. JAFFEE ET AL

2,867,534

TITANIUM BASE ALPHA DISPERSOID ALLOYS

Filed Jan. 23, 1957

3 Sheets-Sheet 3

Fig. 3.

EFFECT OF INCREASING COPPER CONTENT  
ON THE HARDNESS OF Ti-10Sn-BASE ALLOY



INVENTORS.  
ROBERT I. JAFFEE.  
HORACE R. OGDEN.  
BY

Ward, Heath, Haselton, Orme & McElhannon  
ATTORNEYS.

## 1

2,867,534

## TITANIUM BASE ALPHA DISPERSOID ALLOYS

Robert I. Jaffee, Worthington, and Horace R. Ogden, Columbus, Ohio, assignors, by mesne assignments, to Crucible Steel Company of America, Flemington, N. J., a corporation of New Jersey

Application January 23, 1957, Serial No. 635,705

26 Claims. (Cl. 75—175.5)

This invention pertains to alloys of titanium containing as essential constituents at least one of the active eutectoid beta promoters, copper, beryllium, nickel, cobalt and silicon, and at least one promoter of alpha titanium selected from the group consisting of aluminum, tin, antimony and zirconium, characterized by good hot workability, excellent thermal stability and elevated temperature strength, and in being hardened and strengthened in remarkable degree, without undue embrittlement by quenching or cooling at a sufficiently rapid rate from above the critical or eutectoid temperature.

Copper, nickel, cobalt, silicon and beryllium all belong to the group of so-called active eutectoid or compound forming beta promoters. That is to say, these elements when present as alloy additions to titanium, form compounds on cooling from above to below the critical temperature, to produce a microstructure consisting of alpha titanium plus compounds dispersed throughout the alpha matrix.

Of the metals of the active eutectoid beta promoter group, copper is effective over the range of about 0.5 to 20%, nickel and cobalt over the range of about 0.5 to 12% each or in total amount, silicon over the range of about 0.25 to 3% and beryllium over the range of about 0.1 to 2%.

Of the alpha promoters aforesaid, aluminum may range from about 0.5 to 12%, tin from about 0.5 to 23% and antimony from about 0.5 to 19% and zirconium from about 0.5 to 40%, the preferred range being, however, about 0.5 to 20%. The total content of the alpha promoters of this group should be held within limits of about 0.5 to 40%, the proportioning being such that when any one is present on the high side of its range, the total content of the others should be held on the low side or sides of their respective ranges. In these quench hardenable alloys, tin or antimony may be substituted for aluminum in the proportions of about 3% by weight of tin or antimony for 1% of aluminum. The upper limits of fabricability for the alloys of the invention are about 12% for aluminum, 23% for tin and 19% for antimony, 20% for copper, 12% for nickel, 12% for cobalt, 3% for silicon and 2% for beryllium. There is no upper limit for fabricability of zirconium alloying additions to titanium, since zirconium is beta isomorphous with titanium. Zirconium is nevertheless an alpha promoter because alloys of titanium and zirconium always revert to the all-alpha form on cooling to room temperature from the beta field.

Of the interstitial alpha promoter additions, carbon is effective over the range of about 0.05 to 0.5%, oxygen over the range of about 0.05 to 0.4% and nitrogen over the range of about 0.025 to 0.25%. The total content of the interstitials should not exceed about 0.5%, the lower effective limit being about 0.025%.

## 2

The proportioning of the total content of the beta promoters in relation to the alpha promoter additions is preferably such that when the beta promoter content is on the high side, the alpha promoter content should be on the low side and vice versa, of the ranges for each aforesaid.

Preferred ranges for optimum quench hardenability of alloys according to the invention are about: 5 to 8% copper, 4 to 7% nickel, 5 to 8% cobalt, 0.5 to 1.0% silicon, and 0.5 to 1% beryllium, together with about 2 to 4% aluminum, 4 to 8% tin or 4 to 8% antimony.

We have found that the series of alloys above mentioned, particularly those containing copper, have outstanding properties in a number of respects as follows:

- 5 They have improved hot workability as compared to previously known types of titanium base alloys with high-alpha-stabilizer content. They undergo greatly enhanced hardening and strengthening on quenching or rapidly cooling from the beta and alpha-beta temperature ranges.
- 10 They possess excellent elevated temperature strength up to about 1200° F. They have a high modulus of elasticity and a high ratio of modulus of elasticity to density as compared to previously known types of titanium base alloys. They have excellent thermal stability, particularly as annealed below the lower critical temperature, the lower critical temperature being that at which the beta phase transforms on cooling to the alpha phase plus the compounds formed by decomposition of the active eutectoid elements present. For the
- 15 copper-bearing alloys, this compound is  $Ti_2Cu$  which corresponds to  $Fe_3C$  in the iron-carbon phase diagram of steel. This thermal stability results from the fact that the alloy is completely transformed to alpha titanium plus compound. These alloys also possess excellent creep resistance and excellent welding properties.
- 20
- 25
- 30
- 35

The thermally stable conditions for these alloys may be obtained either by slow cooling through the critical temperature range, or by annealing for about  $\frac{1}{4}$  to 24 hours at a temperature below the critical, usually about 50-100° F. below the critical. The longer the annealing cycle the softer the material.

At least half of the total content of active eutectoid beta promoters present in these alloys can be substituted by other stabilizers of beta titanium such as the beta isomorphous or sluggishly eutectoid beta promoters, molybdenum, vanadium, tantalum, columbium, chromium, manganese, iron and tungsten. In this substitution such other beta promoters may be added up to about one-half of their total permissible ranges in the absence of the active eutectoid beta promoter addition. Thus, for example, molybdenum, vanadium, tantalum and columbium may be added up to about 40% to the titanium-aluminum base alloys of the invention in the absence of copper, nickel, cobalt, etc. On the other hand, if the alloy contains, for example, 10% of copper, then metal of the group molybdenum, vanadium, columbium and tantalum may be added up to about 20%, chromium and/or tungsten up to about 12%, manganese up to about 5% and iron up to about 3.5%, as compared to upper limits for these latter additions of up to 25% chromium and/or tungsten, 10% manganese, and 7% iron in the absence of the active eutectoid addition.

These alloys may properly be termed "alpha dispersoid" alloys for reasons above stated, and are basically ternary alloy systems containing one alloy addition such as aluminum, tin, antimony or zirconium, which strengthens the alpha phase, and one active eutectoid

beta promoter addition such as copper, nickel, cobalt, silicon or beryllium, which forms a compound that is insoluble in the service range of these alloys, generally up to 1200° F. More complex alloys of this character can be produced by adding two or more of the active eutectoid beta promoters or two or more of the alpha strengthening elements, for these purposes. The fundamental two-phase alpha plus dispersed compound structure remains unchanged, however.

These alpha dispersoid alloys are particularly adapted for elevated temperature service. As stated, they are usually two-phase alloys, consisting of a strong stable alpha phase and a dispersed compound phase. Superior elevated temperature properties result from the keying effect of the hard dispersed phase.

The hot working methods used in the fabrication of these alloys is of considerable importance, since their properties as heat treated, are controlled to a large extent by the prior fabrication history. There are four temperature regions in which these alloys may be hot worked. Arranged in the order of decreasing temperature, these regions are: (a) the all-beta region, (b) the two-phase, alpha-beta region, (c) the three-phase alpha-beta-compound region, and (d) the two-phase alpha-compound region.

For example, in the case of Ti-Al-Cu alloys of the invention, heat treatment in the all-beta region is carried out in the range of from about 1650° F. up to usually not more than 1800° or 1850° F.; the two-phase alpha-beta region is about 1550-1650° F.; the three-phase alpha-beta-compound region is about 1475° F.; and the two-phase alpha-compound region lies below 1475° F. The ingot breakdown operations for these Ti-Al-Cu alloys are normally performed by hammer forging at about 1800° F. followed by either rolling or swaging at about 1700° F. These alloys are normally given a fairly heavy final reduction of about 60% in area in either the alpha-beta temperature range (1550-1650° F.) or in the alpha-compound range (about 1450° F.) to place the structure in malleable condition for subsequent heat treatment.

The critical temperature for these alloys will vary somewhat with the particular active eutectoid beta promoter addition. For the copper-bearing alloys it is about 1475° F., for the nickel-bearing about 1420° F., for the cobalt-bearing about 1260° F., for the beryllium-bearing about 1550° F. and for the silicon bearing about 1575° F. As stated, for alpha-compound annealing, all of these alloys are annealed at about 50-100° F. below the critical. The beta transus temperature of these alloys also varies somewhat with the alloying content, being the lowest temperature, for any given analysis, above which the alloy is entirely beta. The optimum temperature for beta quenching these alloys is to heat the same to about 50-100° F. above the beta transus and thereupon quench or air cool as discussed below. For the copper-bearing alloys the optimum quenching range for the beta quenched alloys is about 1500-1850° F., and for the optimum quenching from the alpha-beta field, it is about 1580-1610° F. when aluminum is present, and about 1490-1550° F. when tin or antimony is substituted for aluminum.

In these alloys the beta phase formed above the critical temperature transforms completely into martensite and fine eutectoid on rapid quenching, as in water, or into a mixture of alpha titanium and compounds consisting of eutectoid decomposition products on slower cooling from above the critical, as by oil quenching or cooling in air. That is to say, in these alloys the beta phase is not retained on quenching from above the critical, and also the beta transformation is accompanied by marked increase in hardness and tensile strength.

The martensite formed on quenching this type of titanium alloy is quite similar to the martensite formed in

steel on quenching from the austenitizing temperature range. The martensite thus formed on quenching is converted on subsequent tempering in the alpha-compound temperature range, into a microstructure consisting of a fine dispersion of the beta eutectoid decomposition compound, such as  $Ti_2Cu$ , or titanium beryllide, etc., in an alpha titanium matrix. This is similar to the tempering of steel, wherein the martensite formed on the quenching is transformed into a fine dispersion of  $Fe_3C$  in a ferrite matrix.

Relatively high temperatures are required thus to convert the martensite in these titanium alloys, i. e., somewhat under 50-100° F. below the critical. Thus for the copper-bearing alloys the tempering range is about 1000-1400° F., which is quite high as compared to the tempering of steel, the tempering range of which is about 750-1000° F. This tempering of these titanium alloys converts the same to a suitable condition of alpha titanium and dispersed compound, for subsequent service at elevated temperatures.

The high softening temperature of these alloys adapts them for high temperature use in such applications as rotor blades for jet engine compressors, bolts for compressor casings, linings and housings for jet engine combustion chambers, etc.

As an example of the quenched and tempered properties obtainable with these alloys, particularly those containing copper, an analysis comprising about 4% aluminum, 6% copper, balance titanium of commercial purity has, as water quenched from 1580-1600° F., a Vickers hardness of 375, a tensile strength of 190,000 p. s. i., a 0.2% offset yield strength of 130,000 p. s. i., an area reduction of about 30%, a tensile elongation of about 10% and a minimum bend radius of about 4T. This combination of properties has never heretofore been equaled in titanium alloys, in so far as the present applicants are aware. On tempering this alloy at about 1300° F. for about 1 to 16 hours, the Vickers hardness is reduced from 375 to 330-350, with an improvement in bend ductility from 4T as quenched to 3T as tempered. In this condition exceptionally good thermal stability and elevated temperature strength is obtained for service conditions up to about 600-1000° F.

The following Table I shows the effects of the various heat treatments aforesaid on the mechanical properties of a typical alloy according to the invention containing 4% aluminum, 6% copper, balance titanium, as compared to the corresponding binary alloy omitting the alpha promoter, i. e., containing 6% copper, balance titanium.

TABLE I

*The effect of heat treatment on the tensile properties of two alpha-dispersoid alloys*

| Alloy and Heat Treatment     | Tensile Properties of 0.040" sheet; p. s. i. $\times 1,000$ |                   | Percent Elongation in 1" | Percent Reduction in Area |
|------------------------------|-------------------------------------------------------------|-------------------|--------------------------|---------------------------|
|                              | 0.2% Offset Yield                                           | Ultimate Strength |                          |                           |
| Ti-8Cu:                      |                                                             |                   |                          |                           |
| Beta furnace cool            | 85                                                          | 110               | 14                       | 19                        |
| Alpha-compound anneal        | 75                                                          | 100               | 18                       | 19                        |
| Alpha-beta quench            | 130                                                         | 170               | 5                        | 16                        |
| Alpha-beta quench and temper | 90                                                          | 120               | 11                       | 25                        |
| Beta quench                  | 135                                                         | 180               | 4                        | 8                         |
| Beta quench and temper       | 105                                                         | 130               | 11                       | 16                        |
| Ti-4Al-8Cu:                  |                                                             |                   |                          |                           |
| Beta furnace cool            | 130                                                         | 150               | 19                       | 20                        |
| Alpha-compound anneal        | 110                                                         | 120               | 15                       | 30                        |
| Alpha-beta quench            | 150                                                         | 175               | 4                        | 10                        |
| Alpha-beta quench and temper | 135                                                         | 145               | 11                       | 25                        |
| Beta quench                  | 180                                                         | 210               | 7.5                      | 8                         |
| Beta quench and temper       | 180                                                         | 195               | 3                        | 3                         |

The heat treatments referred to in Table I may be elaborated upon to advantage as follows:

(1) *Beta furnace cool heat treatment*.—In this heat treatment, the amount and type of prior work given to the alloy is relatively unimportant. The alloy is heated to some temperature above the beta transus and held at this temperature for a sufficiently long time to insure transformation to an all-beta structure. Following the annealing period, the alloy is slowly cooled through the transformation range, usually by allowing the alloy to cool with the furnace. This treatment results in a structure consisting of a basket-weave alpha pattern surrounded by a coarse alpha-compound eutectoid structure. The amount of the eutectoid varies with composition, some alloys showing islands of alpha, while in others the various alpha particles are closely in contact. The principal advantage of this heat treatment is its relative independence from prior fabrication history.

(2) *Alpha-compound anneal heat treatment*.—The prior fabrication controls the structure of alpha-compound annealed material to a considerable extent. Whenever possible, the alloys are rolled in the alpha-compound region as the final hot-working operation. In some alloys, however, particularly those containing large amounts of aluminum, it is necessary to finish the fabrication in the lower part of the alpha-beta region or in the alpha-beta-compound region due to a compositionally-induced alloy brittleness. The fabrication operations normally serve to break up the compound phase as it forms and to distribute it randomly throughout the matrix. Following the final rolling operations, the alloys are annealed at a temperature just below the eutectoid temperature in order to promote compound agglomeration and to remove any residual cold work from the structure. Following this treatment, the alloys are air cooled. The structure consists of a uniform dispersion of spheroidal compound articles in a fine-grained alpha matrix.

(3) *Alpha-beta quench heat treatment*.—The beta phase of alpha-dispersoid alloys transforms to martensitic alpha or to a very fine eutectoid structure on quenching. Because of the fineness of the structure, it has not been possible to learn the exact nature of the transformation product. The quenched structures have considerably improved strength, but decreased ductility. The purpose of this heat treatment is to develop some of the increased strength resulting from the presence of the martensitic alpha or fine eutectoid while retaining good ductility due to the presence of equiaxed alpha. The final structure is controlled to a considerable extent by the fabrication history. Normally, the alloys are finished in alpha-beta region and air cooled. If sufficient reduction is given in the alpha-beta region, a uniformly fine equiaxed-alpha structure either surrounded by the transformation product or containing islands of the transformation product, depending on composition, is formed. On heat treatment, the alloys are heated to some point in the alpha-beta region and allowed to come to equilibrium. At the annealing temperature, the alloys consist of equiaxed alpha in a matrix of beta. The size and shape of the alpha grains is controlled by the prior fabrication history, while the amount of alpha is controlled by the annealing temperature. At the end of the equilibration period, the alloys are quenched rapidly to room temperature, transforming the beta either to martensitic alpha or to a very fine alpha-compound eutectoid.

(4) *Alpha-beta quench and temper heat treatment*.—Tempering of an alloy quenched from the alpha-beta field promotes decomposition of the martensitic alpha into compound and alpha and spheroidization of the fine

alpha-compound eutectoid. By controlling the tempering conditions, the type of compound structure can be controlled. Thus, it is possible to develop either a very fine structure or one which is comparable to in coarseness that which results from the normal alpha-compound anneal heat treatment. Tempering is normally carried out at some temperature below the eutectoid temperature. Both the amount and distribution of the compound phase are controlled by the quenched structure.

(5) *Beta quench heat treatment*.—In this heat treatment, the alloy is first heated for a sufficient time at some temperature above the beta transus to insure complete transformation to beta and then quenched to room temperature. As in the case of the beta furnace cool heat treatment, the final structure, with the possible exception of grain size, is independent of the fabrication history. The structure of the quenched alloy consists almost entirely of martensitic alpha. If the quench is delayed slightly or if the section size is large, regions containing very fine eutectoid are formed. This heat treatment has the advantages of producing high strengths in most alpha-dispersoid alloys and of being relatively independent of prior fabrication history.

(6) *Beta quench and temper heat treatment*.—Tempering results in much the same structure modification in beta-quenched material as in alpha-beta quenched material. Since the martensitic alpha present in beta-quenched material is of lower alloy content than that present in alpha-beta quenched material (the alloy content of martensitic alpha in a quenched alloy varies inversely with the amount), the compound formed on tempering is usually found principally at the boundaries between the martensitic needles. The tempered beta structures thus far obtained have all contained a relatively fine compound dispersion.

Examination of the data given in Table I above shows that the maximum ductility was obtained when the alloys were given the alpha-compound anneal heat treatment. The beta furnace cooled heat treatment results in a stronger, less ductile structure than the alpha-compound anneal. In the Ti-6Cu alloy, copper functions both as an alpha strengthener and as a compound former. In the

## 50 Ti-4Al-6Cu

alloy, aluminum serves as an alpha strengthener while copper is present chiefly because of its compound-forming ability. Quenching these alloys to form martensitic alpha results in an increase in strength and a decrease in ductility. As would be expected, the increase in strength is greater on quenching from the all-beta region than from the alpha-beta region.

Because of the rapid decomposition of the beta phase of these alloys during cooling, appreciable improvements in properties may also be obtained by heating sufficiently high to form some beta phase, and air cooling. Thus, it is possible to carry out extensive forming operations on the alloy in the soft condition and then harden the formed product by an elevated-temperature anneal followed by air cooling. Such a heat treatment results in only a minimum amount of distortion. The amount of hardening obtained in a given alloy is controlled both by the temperature to which the alloy is heated and by the velocity of the air cool. The effects of this heat treatment on several alpha-dispersoid alloys are shown in the following Table I-A.

TABLE I-A  
*Increase in hardness of several alpha-dispersoid alloys resulting from the air-cool heat treatment*

| Composition (Wt. Percent),<br>Bal. Titanium | Annealing Temperature,<br>°F. | Vickers Hardness Number<br>(10-Kg. Load) |                   |                      |
|---------------------------------------------|-------------------------------|------------------------------------------|-------------------|----------------------|
|                                             |                               | Soft Condition <sup>1</sup>              | After Air Cooling | Increase in Hardness |
| 4Cu.....                                    | 1,600                         | 220                                      | 253               | 33                   |
| 6Cu.....                                    | 1,600                         | 218                                      | 306               | 88                   |
| 8Cu.....                                    | 1,600                         | 226                                      | 401               | 75                   |
| 2Al-6Sn-4Cu-0.1 Be.....                     | 1,600                         | 292                                      | 400               | 108                  |
| 6Sn-4Cu.....                                | 1,600                         | 271                                      | 333               | 62                   |
| 9Sn-4Cu.....                                | 1,500                         | 376                                      | 387               | 11                   |

<sup>1</sup> Normally as alpha-compound annealed.

The following Table I-B shows the effects of various of the heat treatments above discussed on the room temperature mechanical properties of a typical forging alloy according to the invention, having the composition

Ti-7Al-3Cu

TABLE I-B  
*Room temperature tensile properties of a Ti-7Al-3Cu alloy*

[Rolled from  $\frac{1}{2}$ " to  $\frac{3}{4}$ " plate at 1700° F. prior to heat treating as indicated below. Tensile tests in transverse direction.]

| Heat Treatment                                                                                        | Tensile Properties, p. s. i. $\times 1,000$ |                   | Percent Elongation in 1" | Percent Reduction in Area |
|-------------------------------------------------------------------------------------------------------|---------------------------------------------|-------------------|--------------------------|---------------------------|
|                                                                                                       | 0.2% Offset Yield                           | Ultimate Strength |                          |                           |
| 7 hrs. at 1,400° F., air cool.....                                                                    | 122                                         | 135               | 11                       | 11                        |
| 7 hrs. at 1,400° F., air cool plus age <sup>a</sup> .....                                             |                                             | 145               | 8                        | 8                         |
| 7 hrs. at 1,400° F., furnace cool.....                                                                | 132                                         | 144               | 10                       | 8                         |
| 7 hrs. at 1,400° F., furnace cool plus age <sup>a</sup> .....                                         | 140                                         | 148               | 10                       | 9                         |
| 6 hrs. at 1,400° F., plus 24 hrs. at 1,200° F. and air cool to room temp.....                         | 123                                         | 137               | 14                       | 23                        |
| 6 hrs. at 1,400° F., plus 24 hrs. at 1,200° F. and air cool to room temp, plus age <sup>a</sup> ..... | 133                                         | 146               | 16                       | 16                        |
| $\frac{1}{2}$ hr. at 1,700° F., water quench.....                                                     | 132                                         | 164               | 6                        | 25                        |
| $\frac{1}{2}$ hr. at 1,700° F., water quench plus age <sup>a</sup> .....                              | 154                                         | 175               | 4                        | 8                         |
| $\frac{1}{2}$ hr. at 1,700° F., WQ+7:1,400° F., FC <sup>b</sup> .....                                 | 135                                         | 147               | 10                       | 8                         |
| $\frac{1}{2}$ hr. at 1,700° F., WQ+7:1,400° F., FC plus age <sup>a, b</sup> .....                     |                                             | 149               | 8                        | 5                         |
| $\frac{1}{2}$ hr. at 1,700° F., air cool.....                                                         | 133                                         | 150               | 16                       | 14                        |
| $\frac{1}{2}$ hr. at 1,700° F., air cool plus age <sup>a</sup> .....                                  | 147                                         | 152               | 6                        | 8                         |
| $\frac{1}{2}$ hr. at 1,700° F., furnace cool.....                                                     | 137                                         | 148               | 10                       | 8                         |
| $\frac{1}{2}$ hr. at 1,700° F., furnace cool plus age <sup>a</sup> .....                              | 139                                         | 148               | 6                        | 6                         |
| $\frac{1}{2}$ hr. at 1,840° F., water quench.....                                                     | 150                                         | 168               | 0                        | 9                         |
| $\frac{1}{2}$ hr. at 1,840° F., water quench plus age <sup>a</sup> .....                              |                                             | 178               | 2                        | 10                        |
| $\frac{1}{2}$ hr. at 1,840° F., WQ+7:1,400° F., FC <sup>c</sup> .....                                 | 145                                         | 155               | 3                        | 8                         |
| $\frac{1}{2}$ hr. at 1,840° F., WQ+7:1,400° F., FC plus age <sup>a, c</sup> .....                     |                                             | 158               | 4                        | 5                         |
| $\frac{1}{2}$ hr. at 1,840° F., air cool.....                                                         | 133                                         | 150               | 6                        | 8                         |
| $\frac{1}{2}$ hr. at 1,840° F., air cool plus age <sup>a</sup> .....                                  | 140                                         | 149               | 2                        | 2                         |
| $\frac{1}{2}$ hr. at 1,840° F., furnace cool.....                                                     | 124                                         | 126               | 4                        | 6                         |
| $\frac{1}{2}$ hr. at 1,840° F., furnace cool plus age <sup>a</sup> .....                              | 127                                         | 132               | 2                        | 6                         |
| 24 hrs. at 1,200° F., air cool <sup>d</sup> .....                                                     | 134                                         | 148               | 10                       | 11                        |
| 24 hrs. at 1,200° F., air cool plus age <sup>a</sup> .....                                            | 140                                         | 151               | 8                        | 5                         |

<sup>a</sup> Aging heat treatment: 100 hours at 800° F., and air cool.

<sup>b</sup> Dual heat treatment:  $\frac{1}{2}$  hour at 1,700° F. and water quench followed by 7 hours at 1,400° F. and furnace cooling.

<sup>c</sup> Dual heat treatment:  $\frac{1}{2}$  hour at 1,840° F. and water quench followed by 7 hours at 1,400° F. and furnace cooling.

<sup>d</sup> Low temperature anneal.

The following Table II gives the mechanical properties of typical titanium-aluminum-copper alloys in the alpha-compound annealed condition, while Table III gives cor-

responding data for these alloys in the beta quenched condition.

TABLE II  
*Average mechanical properties<sup>1</sup> of Ti-Al-Cu alloys as alpha-compound annealed*

| Composition (Wt. Percent),<br>Bal. Titanium | Tensile Properties, p. s. i. $\times 1,000$ |                   | Percent Elongation in 1" | Percent Reduction in Area | VHN   | MBR <sup>2</sup> |
|---------------------------------------------|---------------------------------------------|-------------------|--------------------------|---------------------------|-------|------------------|
|                                             | 0.2% Offset Yield                           | Ultimate Strength |                          |                           |       |                  |
| 4Cu.....                                    | 65                                          | 83                | 26                       | 48                        | 218   | 0.7              |
| 6Cu.....                                    | 75                                          | 95                | 19                       | 28                        | 232   | 2.1              |
| 2Al.....                                    | 67                                          | 85                | 26                       | 38                        | ----- | -----            |
| 2Al-4Cu.....                                | 84                                          | 98                | 26                       | 46                        | 297   | 2.6              |
| 4Al.....                                    | 86                                          | 99                | 20                       | 45                        | ----- | -----            |
| 4Al-2Cu.....                                | 96                                          | 111               | 15                       | 34                        | 330   | 3.6              |
| 4Al-3Cu.....                                | 91                                          | 102               | 18                       | 40                        | 311   | -----            |
| 4Al-4Cu.....                                | 104                                         | 116               | 18                       | 48                        | 347   | 3.7              |
| 4Al-6Cu.....                                | 114                                         | 124               | 16                       | 34                        | 355   | 4.3              |
| 4Al-8Cu.....                                | 134                                         | 147               | 9                        | 12                        | ----- | -----            |
| 4Al-10Cu.....                               | 134                                         | 154               | 9                        | 13                        | ----- | -----            |
| 6Al-2Cu.....                                | 113                                         | 119               | 15                       | 28                        | ----- | -----            |
| 6Al-2.5Cu.....                              | 122                                         | 129               | 18                       | 27                        | ----- | -----            |
| 6Al-3Cu.....                                | 125                                         | 134               | 12                       | 29                        | ----- | -----            |
| 6Al-4Cu.....                                | 146                                         | 158               | 18                       | 32                        | ----- | -----            |
| 6.5Al-2Cu.....                              | 111                                         | 119               | 14                       | 25                        | ----- | -----            |
| 6.5Al-2.5Cu.....                            | 124                                         | 127               | 10                       | 34                        | ----- | -----            |
| 6.5Al-3Cu.....                              | 135                                         | 140               | 10                       | 28                        | ----- | -----            |
| 7Al-2Cu.....                                | 128                                         | 128               | 11                       | 34                        | ----- | -----            |
| 7Al-3Cu.....                                | 132                                         | 144               | 10                       | 8                         | ----- | -----            |
| 8Al-5Cu.....                                | 158                                         | 169               | 8                        | 8                         | ----- | -----            |
| 6Al-6Sn-3Cu.....                            | 139                                         | 153               | 14                       | 29                        | 372   | -----            |
| 3Al-12Sn-3Cu.....                           | 153                                         | 163               | 14                       | 27                        | 355   | -----            |
| 12Sn-3Cu.....                               | 108                                         | 124               | 14                       | 33                        | ----- | -----            |

<sup>1</sup> Results from both sheet and bar tensile bars included in average. Number of tests vary from one to three.

<sup>2</sup> Minimum bend radius T.

TABLE III  
*Average mechanical properties of Ti-Al-Cu alloys as beta quenched*

| Composition (Wt. Percent),<br>Bal. Titanium | Tensile Properties, p. s. i. $\times 1,000$ |                   | Percent Elongation in 1" | Percent Reduction in Area | VHN   | MBR   |
|---------------------------------------------|---------------------------------------------|-------------------|--------------------------|---------------------------|-------|-------|
|                                             | 0.2% Offset Yield                           | Ultimate Strength |                          |                           |       |       |
| 4Cu.....                                    | 97                                          | 118               | 3                        | 7                         | 328   | 8.5   |
| 6Cu.....                                    | 132                                         | 156               | 2                        | 7                         | 378   | 8.4   |
| 2Al-4Cu.....                                | 117                                         | 135               | 2                        | 7                         | 360   | 4.8   |
| 4Al-2Cu.....                                | 104                                         | 122               | 7                        | 16                        | 317   | 3.0   |
| 4Al-4Cu.....                                | 130                                         | 143               | 7                        | 8                         | 351   | ----- |
| 4Al-6Cu.....                                | 179                                         | 190               | 4                        | 8                         | 419   | ----- |
| 4Al-8Cu.....                                | 205                                         | 211               | 3                        | 3                         | ----- | ----- |
| 4Al-10Cu.....                               |                                             | 113               | 0                        | -----                     | 409   | ----- |

\*Broke in grips before yield.

The data in Table II shows that the strength-elongation characteristics of the Ti-Al-Cu alloys, as alpha-compound annealed, are dependent primarily on the total alloy content, with increased total alloy content resulting in increased strength and decreased ductility. The bend properties, hardness, yield strength and reduction in area values support the conclusion that increasing the alloy content results in a uniform increase in strength and a decrease in ductility.

Comparison of the data for the beta quenched Ti-Al-Cu alloys as given in Table III with the values for these alloys in the alpha-compound annealed condition as given in Table II, reveals that only the most highly alloyed samples had strength-elongation properties as beta quenched which were comparable to those of the alpha-compound annealed material. The difference between the two heat treated conditions is greater for these alloys having a smaller total alloy content.

It can thus be concluded that quenching or quenching

and tempering heat treatments will be advantageous only for the most highly alloyed systems of this series.

The excellent elevated temperature properties, i. e., at 1000° F., of the Ti-Al-Cu alloys, as alpha-compound annealed, are shown by the test results given in the following Table IV.

TABLE IV

*Elevated temperature (1000° F.)<sup>1</sup> tensile properties of Ti-(Al, Sb, Sn)Cu alloys as alpha-compound annealed*

| Composition (Wt. Percent),<br>Bal. Titanium | Tensile Properties,<br>p. s. i. $\times 1,000$ |                      | Percent<br>Elongation<br>in 1" | Percent<br>Reduction<br>in<br>Area |
|---------------------------------------------|------------------------------------------------|----------------------|--------------------------------|------------------------------------|
|                                             | Est.<br>Yield                                  | Ultimate<br>Strength |                                |                                    |
| 4Cu                                         | 30                                             | 36                   | 65                             | 98                                 |
| 6Cu                                         | 38                                             | 41                   | 30                             | 91                                 |
| 2Al-4Cu                                     | 40                                             | 47                   | 34                             | 83                                 |
| 4Al                                         |                                                | 52                   | 21                             | 73                                 |
| 4Al-2Cu                                     | 20                                             | 37                   | 40                             | 94                                 |
| 4Al-4Cu                                     | 50                                             | 60                   | 46                             | 82                                 |
| 4Al-6Cu                                     | 55                                             | 72                   | 36                             | 90                                 |
| 4Al-8Cu                                     | 57                                             | 83                   | 35                             | 74                                 |
| 4Al-10Cu                                    | 58                                             | 77                   | 45                             | 87                                 |
| 4Al-12Cu                                    |                                                | 65                   |                                |                                    |
| 6Al-2Cu                                     | 62                                             | 82                   | 50                             | 68                                 |
| 6Al-4Cu                                     | 68                                             | 84                   | 52                             | 84                                 |
| 6Al-6Cu                                     | 82                                             | 103                  | 40                             | 74                                 |
| 8Al-2Cu                                     | 69                                             | 99                   | 45                             | 49                                 |
| 8Al-4Cu                                     | 77                                             | 96                   | 55                             | 83                                 |
| 8Al-5Cu                                     | 84                                             | 109                  | 45                             | 70                                 |
| 8Al-6Cu                                     | 96                                             | 1.2                  | 40                             | 66                                 |
| 10Al-2Cu                                    | 88                                             | 125                  |                                | 20                                 |
| 10Al-4Cu                                    | 87                                             | 126                  | 30                             | 53                                 |
| 10Al-6Cu                                    | 93                                             | 118                  | 50                             | 75                                 |
| 12Al-6Cu                                    |                                                | 98                   | 28                             | 25                                 |
| 12Al-8Cu                                    | 64                                             | 107                  | 5                              | 15                                 |
| 6Sb-4Cu                                     |                                                | 73                   | 33                             | 61                                 |
| 12Sb-4Cu                                    |                                                | 86                   | 19                             | 55                                 |
| 15Sb-4Cu                                    |                                                | 112                  | 3                              | 3                                  |
| 12Sb-4Cu                                    |                                                | 63                   | 24                             | 61                                 |
| 15Sb-4Cu                                    |                                                | 80                   | 23                             | 64                                 |

<sup>1</sup> Both bar and sheet test specimens were used. Most values given are from a single test specimen.

From the foregoing data of Table IV, alloying is seen to result in a marked increase in elevated temperature tensile strength. The beneficial effects of copper are shown to be quite dependent on the alpha promoter or aluminum content. At low aluminum contents the addition of copper results in a large improvement in elevated temperature strength. As the amount of aluminum is increased, however, the addition of copper is less beneficial. For example, an alloy containing about 2 to 4% by weight of aluminum, is improved with copper additions up to 10%, while in an alloy containing 10% aluminum, more than 4% copper results in a reduction in elevated temperature strength. Since binary titanium-aluminum alloys containing moderate amounts of aluminum are difficult to fabricate, the beneficial effects of copper additions thereto on elevated temperature strength will be particularly advantageous in wrought alloys of this series.

In order to obtain information on the thermal stability of Ti-Al-Cu alpha dispersoid alloys after various heat treatments, they were exposed to 800° F. for 24 hours and the hardness and bend properties re-determined. The effect of this elevated temperature exposure is shown by the data in the following Table V. From this data it will be seen that the quenched alloys were unstable, as would be expected. The alpha-compound annealed and beta quenched and tempered conditions were found to be the most stable. These results also indicate that a considerable amount of compound precipitation occurred during the thermal exposure in the alpha-beta quenched and tempered alloys.

TABLE V

*Effects of aging 24 hours at 800° F. on hardness and bend properties of Ti-Al-Cu alloys*

| Alloy      | Heat Treatment           | As Heat Treated        |                    | Change on aging 24 hrs. at 800° F. |                    |
|------------|--------------------------|------------------------|--------------------|------------------------------------|--------------------|
|            |                          | VHN,<br>10-kg.<br>load | MBR,<br>T<br>long. | VHN,<br>10-kg.<br>load             | MBR,<br>T<br>long. |
| Ti-2Al-4Cu | Alpha-compound anneal.   | 297                    | 2.6                | +15                                | +0.2               |
| Ti-4Al-4Cu | do                       | 347                    | 3.6                | -5                                 | -0.2               |
| Ti-4Al-2Cu | do                       | 330                    | 3.6                | +10                                | -0.6               |
| Average    | do                       | 325                    | 3.3                | +7                                 | -0.2               |
| Ti-2Al-4Cu | Alpha-beta quench        | 353                    | 4.6                | +11                                | +0.7               |
| Ti-4Al-4Cu | do                       | 385                    | 4.4                | +50                                | +5.6               |
| Ti-4Al-2Cu | do                       | 361                    | 2.8                | +3                                 | -0.2               |
| Average    | do                       | 366                    | 3.9                | +21                                | +2.0               |
| Ti-2Al-4Cu | Alpha beta quench+temper | 328                    | 4.2                | +47                                | +1.0               |
| Ti-4Al-4Cu | do                       | 385                    | 8.3                | +18                                | +1.3               |
| Ti-4Al-2Cu | do                       | 340                    | 3.6                | +44                                | +0.4               |
| Average    | do                       | 351                    | 5.4                | +36                                | +0.9               |
| Ti-2Al-4Cu | Beta quench              | 360                    | 5.0                | +12                                | +5.0               |
| Ti-4Al-4Cu | do                       | 351                    | 3.4                | +55                                | +6.6               |
| Ti-4Al-2Cu | do                       | 317                    | 3.0                | +37                                | +1.6               |
| Average    | do                       | 343                    | 3.8                | +35                                | +4.4               |
| Ti-2Al-4Cu | Beta quench + temper     | 385                    | 9.4                | -11                                | +0.4               |
| Ti-4Al-4Cu | do                       | 369                    | 10.0               | +18                                | 0.0                |
| Ti-4Al-2Cu | do                       | 362                    | 3.1                | +22                                | 0.0                |
| Average    | do                       | 372                    | 7.5                | +10                                | +0.1               |

The results of stress-rupture tests on the Ti-Al-Cu alloys are shown in the following Table VI. Examination of this data shows that increasing the copper content considerably improves the stress-rupture properties of these alloys, and that extremely good stress-rupture properties are obtained for copper additions of about 8% and over.

TABLE VI

Results of stress-rupture tests on Ti-Al-Cu alloys as alpha-compound annealed

| Composition (Wt. Percent), Bal. Titanium | Test Temperature, °F. | Applied Stress, p. s. i. | Rupture Time, Hrs.        | Percent Elongation |
|------------------------------------------|-----------------------|--------------------------|---------------------------|--------------------|
| 6Cu.....                                 | 800                   | 80,000                   | Broke on loading.         | 15.5               |
| 4Al-6Cu.....                             | 800                   | 80,000                   | 16.1.....                 | 14.7               |
| 4Al-6Cu.....                             | 800                   | 75,000                   | 48.....                   | 23.0               |
| 4Al-8Cu.....                             | 800                   | 80,000                   | 150.1.....                | 5.5                |
| 4Al-10Cu.....                            | 800                   | 80,000                   | >362.0 <sup>1</sup> ..... | >6.8               |

<sup>1</sup> Test discontinued after 362 hours.

The effect of substituting the alpha promoters tin and antimony for all or part of aluminum in the copper-bearing alpha dispersoid alloys is shown by the test results in the following Tables VII, VIII and IX.

TABLE VII

Average mechanical properties of Ti-Cu—plus Al,Sn,Sb alloys

AS ALPHA-COMPOUND ANNEALED

| Composition (Wt. Percent), Bal. Titanium | Tensile properties, p. s. i. $\times 1,000$ |                   | Percent Elongation in 1" | Percent Reduction in Area | VHN   | MBR   |
|------------------------------------------|---------------------------------------------|-------------------|--------------------------|---------------------------|-------|-------|
|                                          | 0.2% Offset Yield                           | Ultimate Strength |                          |                           |       |       |
| 4Cu-6Sn.....                             | 87                                          | 98                | 20                       | 46                        | 277   | 2.1   |
| 6Cu-6Sn.....                             | 90                                          | 112               | 14                       | 25                        | ..... | ..... |
| 6Cu-6Sb.....                             | 97                                          | 119               | 10                       | 16                        | ..... | ..... |
| 4Cu-4Al-4Sn.....                         | 124                                         | 146               | 13                       | 25                        | 366   | 5.6   |
| 4.5Cu-2Al-3Sn.....                       | 101                                         | 113               | 6                        | 17                        | 310   | 6.6   |
| 4Cu-2Al-3Sn-0.1Be.....                   | 97                                          | 113               | 12                       | 19                        | 294   | 1.5   |
| 6Sn-4Al-4Cu.....                         | 131                                         | 143               | 10                       | 14                        | ..... | ..... |
| 6Sb-4Al-4Cu.....                         | 131                                         | 138               | 11                       | 11                        | ..... | ..... |
| 9Sn-3Al-4Cu.....                         | 124                                         | 136               | 13                       | 26                        | ..... | ..... |
| 9Sb-3Al-4Cu.....                         | 107                                         | 111               | 17                       | 33                        | ..... | ..... |
| 9Sb-3Al-4Cu.....                         | 126                                         | 142               | 7                        | 15                        | ..... | ..... |
| 12Sn-2Al.....                            | 95                                          | 108               | 20                       | 38                        | ..... | ..... |
| 12Sn-2Al-4Cu.....                        | 132                                         | 142               | 12                       | 18                        | ..... | ..... |
| 12Sb-2Al.....                            | 106                                         | 110               | 18                       | 30                        | ..... | ..... |
| 12Sb-2Al-4Cu.....                        | 132                                         | 140               | 14                       | 23                        | ..... | ..... |
| 15Sn-1Al.....                            | 99                                          | 107               | 17                       | 39                        | ..... | ..... |
| 15Sn-1Al-4Cu.....                        | 135                                         | 144               | 17                       | 26                        | ..... | ..... |
| 15Sb-1Al.....                            | 109                                         | 112               | 16                       | 29                        | ..... | ..... |

AS BETA QUENCHED

|                  |     |     |   |    |       |       |
|------------------|-----|-----|---|----|-------|-------|
| 4Cu-6Sn.....     | 121 | 146 | 2 | 3  | 370   | 5.7   |
| 6Cu-6Sn.....     | 151 | 195 | 6 | 18 | 430   | 7.6   |
| 6Cu-6Sb.....     | 140 | 184 | 4 | 12 | 388   | 7.1   |
| 4Cu-4Al-4Sn..... | 151 | 170 | 5 | 13 | ..... | ..... |

ELEVATED TEMPERATURE (1,000° F.) TENSILE PROPERTIES AS ALPHA-COMPOUND ANNEALED

|                  |    |    |    |    |       |       |
|------------------|----|----|----|----|-------|-------|
| 4Cu-4Al-4Sn..... | 63 | 82 | 40 | 87 | ..... | ..... |
| 6Cu-10Sb.....    | 50 | 66 | 48 | 67 | ..... | ..... |

TABLE VIII

Effect of aging 24 hours at 800° F. on the hardness and bend properties of Ti-Cu—plus Al,Sn alloys as alpha-compound annealed

| Composition (Wt. Percent), Bal. Titanium | Before Aging |     | Increase on Aging |     |
|------------------------------------------|--------------|-----|-------------------|-----|
|                                          | MBR          | VHN | MBR               | VHN |
| 4Cu-6Sn.....                             | 2.1          | 277 | 0.3               | -5  |
| 4Cu-4Al-4Sn.....                         | 6.8          | 366 | 0.4               | -62 |
| 4Cu-2Al-3Sn-0.1Be.....                   | 1.5          | 294 | 2.7               | 26  |

TABLE IX

Results of stress-rupture tests on a Ti-Cu—plus Al,Sn alloys as alpha-compound annealed

| Composition (Wt. Percent), Bal. Titanium | Test Temperature, °F. | Applied Stress, p. s. i. | Rupture Time, hrs.  | Percent Elongation |
|------------------------------------------|-----------------------|--------------------------|---------------------|--------------------|
| 4Cu-4Al-4Sn.....                         | 800                   | 80,000                   | <sup>1</sup> >407.8 | .....              |
| (1).....                                 | 800                   | 85,000                   | <sup>1</sup> >232.5 | 0.67               |
| (1).....                                 | 800                   | 95,000                   | <sup>1</sup> >343   | 4.6                |

<sup>1</sup> These results from one specimen. After 407.8 hours at 80,000 p. s. i. the stress was raised to 85,000 p. s. i. After 232.5 hours at 85,000 p. s. i., the stress was raised to 90,000 p. s. i. The test was discontinued after 343 hours at 95,000 p. s. i.

These data show that tin or antimony may be substituted for aluminum on a replacement basis of about 3% of the former for 1% of the latter, on a generally comparable basis as regards properties of the resulting alloy. A definite increase in density results from such substitution of tin or antimony for aluminum. However, such substitution does improve fabricability somewhat, tin being superior to antimony in this respect.

The alpha-compound annealed properties of these Sn, Sb alpha substituted alloys, are shown to be reasonably analogous to the Ti-Al-Cu alloys in the same condition of heat treatment. Here again tin appears to be slightly superior to antimony in its effect. Such alpha substituted alloys are shown to have in the beta quenched condition approximately the same mechanical property levels as the equivalent Ti-Al-Cu alloys, and this same equivalency is shown to hold at elevated temperatures also. The stress-rupture tests show that even further improvement in stress-rupture properties is obtained by increasing the aluminum equivalent, alpha strengthener content above 4%. The aging tests show that these alpha substituted alloys have good thermal stability in the alpha-compound annealed condition.

The effect of replacing all or part of the copper in the alpha dispersoid copper-bearing alloys above discussed by the other compound formers beryllium, nickel, cobalt and silicon, is shown in the following Tables X to XIII,

inc., which also show the effect of replacing part of the copper with the relatively sluggishly eutectoid element manganese.

TABLE X

Average mechanical properties of Ti—Al—plus Cu, Be, Ni, Co, Si alloys as alpha-compound annealed

| Composition (Wt. Percent), Bal. Titanium | Tensile Properties, p. s. i. $\times 1,000$ |                   | Percent Elongation in 1" | Percent Reduction in Area | VHN | MBR, T | 10 |
|------------------------------------------|---------------------------------------------|-------------------|--------------------------|---------------------------|-----|--------|----|
|                                          | 0.2% Offset Yield                           | Ultimate Strength |                          |                           |     |        |    |
| 0.1Be.....                               | 68                                          | 74                | 26                       | 51                        | 163 | 1.2    |    |
| 0.25Be.....                              | 58                                          | 80                | 19                       | 31                        | 158 | 1.1    |    |
| 0.5Be.....                               | 52                                          | 72                | 29                       | 46                        | 188 | 0.25   |    |
| 2Al-0.1Be.....                           | 65                                          | 83                | 20                       | 39                        | 218 | 1.4    |    |
| 2Al-0.25Be.....                          | 76                                          | 95                | 17                       | 31                        | 226 | 2.1    |    |
| 2Al-0.5Be.....                           | 70                                          | 86                | 28                       | 44                        | 264 | 2.1    | 25 |
| 4Al-0.1Be.....                           | 84                                          | 96                | 17                       | 27                        | 256 | 2.3    |    |
| 4Al-0.2Be.....                           | 84                                          | 96                | 20                       | 42                        | 297 | 2.6    |    |
| 4Al-0.25Be.....                          | 84                                          | 98                | 20                       | 32                        | 254 | 2.2    |    |
| 4Al-0.5Be.....                           | 88                                          | 104               | 16                       | 24                        | 258 | 2.3    |    |
| 4Al-4Co.....                             | 117                                         | 136               | 10                       | 10                        | 335 | 5.4    |    |
| 4Al-6Co.....                             | 127                                         | 146               | 9                        | 12                        | 356 | 3.8    |    |
| 4Al-4Ni.....                             | 96                                          | 107               | 6                        | 16                        | 316 | 6.8    | 30 |
| 4Al-6Ni.....                             | 108                                         | 122               | 4                        | 12                        | 331 | 8.7    |    |
| 4Al-0.5Si.....                           | 103                                         | 116               | 14                       | 25                        |     |        |    |
| 4Al-1Si.....                             | 95                                          | 106               | 16                       | 38                        | 317 | 2.4    |    |
| 2Al-3.9Cu-0.15Be.....                    | 97                                          | 113               | 10                       | 18                        | 322 | 4.6    |    |
| 4Al-5Cu-1Mn.....                         | 128                                         | 135               | 15                       | 37                        | 372 | 2.8    |    |

TABLE XI

Average mechanical properties of Ti—Al—plus Cu, Be, Co, Ni, Si alloys as beta quenched

| Composition (Wt. Percent), Bal. Titanium | Tensile Properties, p. s. i. $\times 1,000$ |                   | Percent Elongation in 1" | Percent Reduction in Area | VHN | MBR, T  | 35 |
|------------------------------------------|---------------------------------------------|-------------------|--------------------------|---------------------------|-----|---------|----|
|                                          | 0.2% Offset Yield                           | Ultimate Strength |                          |                           |     |         |    |
| 0.1Be.....                               | 67                                          | 88                | 17                       | 21                        | 191 | 0.8     |    |
| 0.25Be.....                              | 80                                          | 99                | 8                        | 8                         | 273 | 4.8     |    |
| 0.5Be.....                               | 80                                          | 96                | 8                        | 10                        | 272 | 2.5     |    |
| 2Al-0.1Be.....                           | 84                                          | 108               | 6                        | 12                        | 260 | 1.4     |    |
| 2Al-0.25Be.....                          | 99                                          | 120               | 6                        | 15                        | 268 | 3.0     |    |
| 2Al-0.5Be.....                           | 96                                          | 111               | 8                        | 10                        | 330 | 5.0     |    |
| 4Al-0.1Be.....                           | 91                                          | 114               | 11                       | 24                        | 255 | 2.2     |    |
| 4Al-0.2Be.....                           | 105                                         | 116               | 11                       | 15                        | 311 | 3.3     |    |
| 4Al-0.25Be.....                          | 113                                         | 133               | 4                        | 8                         | 303 | 4.0     |    |
| 4Al-0.5Be.....                           | 132                                         | 152               | 2                        | 7                         | 382 | $>10.0$ |    |
| 0.5Si.....                               |                                             |                   |                          |                           | 193 | 0       |    |
| 1.0Si.....                               |                                             |                   |                          |                           | 215 | 1.0     |    |
| 1.5Si.....                               |                                             |                   |                          |                           | 227 | 1.5     |    |
| 5Cu-0.5Be.....                           |                                             |                   |                          |                           | 473 | $>10.0$ |    |
| 2Al-5Cu-0.5Be.....                       | 198                                         | 204               | 1                        | 3                         | 473 | $>10.0$ |    |
| 4Al-5Cu-1Mn.....                         |                                             |                   |                          |                           | 469 | $>10.0$ |    |
| 3Cu-1.0Si.....                           |                                             |                   |                          |                           | 291 | 3.1     |    |
| 5Cu-0.5Si.....                           |                                             |                   |                          |                           | 359 | 6.0     |    |
| 2Al-3Cu-1Si.....                         |                                             |                   |                          |                           | 354 | 5.5     |    |
| 2Al-5Cu-0.5Si.....                       |                                             |                   |                          |                           | 377 | 5.3     |    |
| 4Al-0.5Be*.....                          | 98                                          | 122               | 8                        | 7                         | 275 | 4.8     |    |
| 4Al-4Co*.....                            |                                             |                   |                          |                           | 382 | 3.2     |    |
| 4Al-6Co*.....                            |                                             |                   |                          |                           | 400 | 4.4     |    |
| 4Al-4Ni*.....                            |                                             |                   |                          |                           | 433 | 8.8     |    |
| 4Al-6Ni*.....                            |                                             |                   |                          |                           | 446 | 9.2     |    |
| 3.9Cu-0.15Be*.....                       | 123                                         | 181               | 12                       | 25                        | 433 | 5.6     |    |
| 4Al-5Cu-1Mn*.....                        | 133                                         | 184               | 12                       | 22                        | 381 | 2.6     |    |
| 2Al-0.5Si*.....                          |                                             |                   |                          |                           | 236 | 1.8     |    |
| 2Al-1.0Si*.....                          |                                             |                   |                          |                           | 326 | 2.4     |    |

\*These samples quenched from the alpha-beta field.

TABLE XII  
14

Elevated temperature (1000° F.) tensile properties of Ti—Al—plus Cu, Be, Ni, Co, Si alloys as alpha-compound annealed

| Composition (Wt. Percent) Bal. Titanium | Tensile Properties, p. s. i. $\times 1,000$ |                   | Percent Elongation in 1" | Percent Reduction in Area | 5 |
|-----------------------------------------|---------------------------------------------|-------------------|--------------------------|---------------------------|---|
|                                         | Est. Yield Strength                         | Ultimate Strength |                          |                           |   |
| 0.5Be.....                              | 17                                          | 22                | 55                       | 83                        |   |
| 2Al-0.5Be.....                          | 22                                          | 36                | 46                       | 74                        |   |
| 4Al-4Co.....                            |                                             | 55                | 44                       | 90                        |   |
| 4Al-6Co.....                            |                                             | 57                | 44                       | 87                        |   |
| 10Al-5Co.....                           | 43                                          | 81                | 5                        | 5                         |   |
| 4Al-4Ni.....                            |                                             | 47                | 42                       | 64                        |   |
| 4Al-6Ni.....                            |                                             | 53                | 53                       | 84                        |   |
| 10Al-5Ni.....                           | 59                                          | 79                | 15                       | 30                        |   |
| 4Al-0.5Si.....                          |                                             | 60                | 26                       | 57                        |   |
| 4Al-5Cu-1Mn.....                        |                                             | 76                | 46                       | 97                        |   |
| For comparison:                         |                                             |                   |                          |                           |   |
| 4Al-4Cu.....                            | 50                                          | 60                | 46                       | 82                        |   |
| 4Al-6Cu.....                            | 55                                          | 72                | 36                       | 90                        |   |
| 8Al-4Cu.....                            |                                             | 96                | 30                       | 83                        |   |
| 10Al-4Cu.....                           |                                             | 126               | 30                       | 53                        |   |

TABLE XIII

Effect of aging 24 hours at 800° F. on the hardness and bend properties of alpha-compound annealed Ti—Al—plus Cu, Be, Ni, Co, Si alloys

| Composition (Wt. Percent), Bal. Titanium | Before Aging |     | Increase Due to Aging |     | 40 |
|------------------------------------------|--------------|-----|-----------------------|-----|----|
|                                          | MBR          | VHN | MBR                   | VHN |    |
| 2Al-0.5Be.....                           | 2.5          | 241 | -0.5                  | +20 |    |
| 4Al-0.2Be.....                           | 2.4          | 272 | +0.1                  | -78 |    |
| 4Al-1Si.....                             | 2.4          | 317 | +1.9                  | -25 |    |
| 4Al-4Ni.....                             | 6.5          | 316 | -0.6                  | -52 |    |
| 4Al-6Ni.....                             | 9.4          | 331 | +0.6                  | -2  |    |
| 4Al-4Co*.....                            | 5.9          | 335 | +4.1                  | +13 |    |
| 4Al-6Co*.....                            | 2.8          | 356 | +7.2                  | +55 |    |
| 4Al-5Cu-1Mn.....                         | 2.8          | 372 | +3.7                  | -21 |    |

\*May have been annealed in alpha-beta-compound field instead of alpha-compound field.

Referring to the mechanical properties for these alloys in the alpha-compound annealed condition, as given in Table X, it will be seen that all of these alloys except Ti—Al—Ni and Ti—Al—Cu—Be are found to be equivalent to the Ti—Al—Cu alloys. The Ti—Al—Be and Ti—Al—Si alloys are shown to be equivalent to the low alloy Ti—Al—Cu alloys, while the Ti—Al—Co and Ti—Al—Cu—Mn alloys are shown to be equivalent to the high alloy Ti—Al—Cu alloys.

Referring to the beta-quenched properties of Table XI, it will be seen that all of these alloys undergo quench hardening, the Ti—Al—Be and Ti—Al—Si alloys less so than the alloys containing nickel, cobalt and manganese. The combination of high hardness and good bend properties exhibited by the Ti—Al—Co alloys as quenched, appears particularly promising.

With respect to the elevated temperature tensile properties of Table XII, it will be seen that on an equal weight basis, both cobalt and nickel are somewhat inferior to copper in their effect on elevated temperature properties. The addition of a small amount of manganese is beneficial in this regard. The Ti—4Al—0.5Si alloy compares favorably with the Ti—4Al—4Cu alloy in strength but not in ductility.

The aging tests of Table XIII show that the Ti—Al—Be, Ti—Al—Si and Ti—Al—Ni alloys possess reasonably good thermal stability. The Ti—Al—Co and Ti—Al—Mn alloys, however, show definite indications of

instability. These results indicate that manganese promotes the retention of the beta phase due to its beta stabilizing characteristics.

The foregoing test results indicate that neither silicon nor beryllium can completely replace copper in alpha dispersoid alloys, since the total amount which can be added is small. The replacement of a small part of the copper

by manganese results in a slight improvement in properties as compared to the corresponding Ti-Al-Cu alloys, but the manganese-containing alloys are not thermally stable.

Room temperature mechanical properties of other alloys 5 according to the invention, as rolled and annealed at about 1550° F., are given in the following Table XIV:

TABLE XIV  
*Mechanical properties of Ti-(Al, Sb, Sn)-(Cu, Be)  
alloys as annealed*  
(COMMERCIAL PURITY Ti-BASE)

| Al | Cu  | Other  | Tensile Properties,<br>p. s. i. $\times 1,000$ |                      | Percent<br>Elong-<br>ation<br>in 1" | Min.<br>Bend, T<br>Long. | Vickers<br>Hardness |
|----|-----|--------|------------------------------------------------|----------------------|-------------------------------------|--------------------------|---------------------|
|    |     |        | 0.2%<br>Offset<br>Yield                        | Ultimate<br>Strength |                                     |                          |                     |
| 5  | 0.5 |        | 97                                             | 101                  | 22                                  | 2.5                      | 334                 |
| 5  | 1   |        | 110                                            | 117                  | 20                                  | 2.5                      | 316                 |
| 5  | 1.5 |        | 107                                            | 115                  | 20                                  | 2.5                      | 305                 |
| 5  | 1.5 | 0.1C   | 114                                            | 122                  | 18                                  | 2.7                      | 318                 |
| 5  | 2   | 0.1C   | 110                                            | 119                  | 16                                  | 2.5                      | 312                 |
| 5  | 3   | 0.1C   | 123                                            | 133                  | 12                                  | 2.4                      | 354                 |
| 5  | 5   | 0.1C   | 141                                            | 152                  | 12                                  | 5.1                      | 347                 |
| 5  | 0.5 | 0.1C   | 127                                            | 130                  | 14                                  | 1.7                      | 341                 |
| 5  | 1   | 0.1C   | 126                                            | 132                  | 17                                  | 2.4                      | 325                 |
| 5  | 1.5 | 0.1C   | 129                                            | 135                  | 17                                  | 2.3                      | 343                 |
| 5  | 2   | 0.1C   | 130                                            | 135                  | 15                                  | 4.9                      | 350                 |
| 5  | 3   | 0.1C   | 140                                            | 147                  | 13                                  | 4.9                      | 378                 |
| 5  | 5   | 0.1C   | 147                                            | 156                  | 11                                  | Br                       | 375                 |
| 5  | 0.5 | 0.2C   | 127                                            | 136                  | 19                                  | 2.5                      | 363                 |
| 5  | 1   | 0.2C   | 132                                            | 137                  | 16                                  | 2.3                      | 357                 |
| 5  | 1.5 | 0.2C   | 120                                            | 129                  | 19                                  | 1.7                      | 371                 |
| 5  | 2   | 0.2C   | 142                                            | 149                  | 12                                  | 5.2                      | 364                 |
| 5  | 3   | 0.2C   | 153                                            | 153                  | 10                                  | Br                       | 353                 |
| 5  | 5   | 0.2C   | 153                                            | 160                  | 3                                   | Br                       | 372                 |
| 5  | 0.5 | 0.25C  | 140                                            | 141                  | 12                                  | 1.7                      | 346                 |
| 5  | 1   | 0.25C  | 136                                            | 139                  | 15                                  | 2.5                      | 334                 |
| 5  | 1.5 | 0.25C  | 139                                            | 145                  | 14                                  | 2.5                      | 343                 |
| 5  | 2   | 0.25C  | 138                                            | 143                  | 10                                  | 5.1                      | 376                 |
| 5  | 3   | 0.25C  | 139                                            | 149                  | 9                                   | Br                       | 388                 |
| 5  | 0.5 | 0.1O   | 113                                            | 118                  | 14                                  | 2.4                      | 350                 |
| 5  | 1   | 0.1O   | 121                                            | 130                  | 14                                  | 2.3                      | 343                 |
| 5  | 1.5 | 0.1O   | 122                                            | 130                  | 17                                  | 2.7                      | 369                 |
| 5  | 2   | 0.1O   | 126                                            | 136                  | 14                                  | 4.8                      | 349                 |
| 5  | 0.5 | 0.2O   | 129                                            | 139                  | 17                                  | 2.4                      | 354                 |
| 5  | 1   | 0.2O   | 127                                            | 136                  | 16                                  | 2.5                      | 385                 |
| 5  | 1.5 | 0.2O   | 126                                            | 134                  | 14                                  | 3.6                      | 380                 |
| 5  | 2   | 0.2O   | 133                                            | 140                  | 11                                  | 4.9                      | 364                 |
| 5  | 0.5 | 0.10N  | 129                                            | 135                  | 18                                  | 2.5                      | 346                 |
| 5  | 1.5 | 0.09N  | 131                                            | 134                  | 12                                  | 2.6                      | 375                 |
| 5  | 0.5 | 0.18N  | 132                                            | 139                  | 13                                  | 2.3                      | 370                 |
| 5  | 1   | 0.18N  | 142                                            | 146                  | 11                                  | 5.2                      | 383                 |
| 5  | 1.5 | 0.17N  | 129                                            | 141                  | 1                                   | 6.1                      | 390                 |
| 4  | 2.5 | 5Cb    | 124                                            | 134                  | 9                                   | 3.4                      | 349                 |
| 4  | 2.5 | 2.5Cr  | 141                                            | 146                  | 5                                   | 6.7                      | 347                 |
| 4  | 2.5 | 1.5Fe  | 114                                            | 134                  | 12                                  | 2.8                      | 344                 |
| 4  | 2.5 | 2.5Mn  | 120                                            | 139                  | 8                                   | 3.7                      | 361                 |
| 4  | 2.5 | 2.5Mo  | 129                                            | 136                  | 8                                   | 3.5                      | 333                 |
| 4  | 2.5 | 2Ni    | 113                                            | 130                  | 5                                   | 3.9                      | 343                 |
| 4  | 2.5 | 5Ta    | 110                                            | -----                | 11                                  | 4.1                      | 350                 |
| 4  | 2.5 | 5V     | 133                                            | 139                  | 1                                   | 3.6                      | 346                 |
| 4  | 2.5 | 2.5W   | 123                                            | 134                  | 9                                   | 3.6                      | 344                 |
| 5  | --- | 0.25Be | 84                                             | 98                   | 11                                  | -----                    | 311                 |
| 5  | --- | 1Be    | 95                                             | 110                  | 7                                   | -----                    | 349                 |

(IODIDE Ti-BASE)

| Al  | Sn  |              |     |     |    |     |     |
|-----|-----|--------------|-----|-----|----|-----|-----|
| 5   | 2.5 | 0.5Cu-0.25C  | 144 | 156 | 12 | 4.1 | 404 |
| 5   | 2.5 | 1Cu-0.25C    | 133 | 133 | 11 | 2.5 | 407 |
| 5   | 2.5 | 1.5Cu-0.25C  | 134 | 134 | 10 | 3.6 | 424 |
| 5   | 2.5 | 0.1Be-0.25C  | 133 | 133 | 22 | 4.0 | 396 |
| 5   | 2.5 | 0.25Be-0.25C | 137 | 139 | 10 | 3.8 | 400 |
| --- | 5   | 1Cu          | 55  | 72  | 19 | 3.1 | 269 |
| --- | 10  | 1Cu          | 75  | 94  | 15 | 2.0 | 276 |
| --- | 15  | 1Cu          | 100 | 112 | 9  | 2.9 | 322 |
| --- | 10  | 1Cu-0.1O     | 98  | 108 | 22 | 1.9 | 340 |
| --- | 10  | 1Cu-0.1O     | 94  | 108 | 14 | 3.4 | 347 |
| --- | 10  | 1Cu-0.1N     | 114 | 128 | 11 | 6.3 | 375 |

(COMMERCIAL PURITY Ti-BASE)

|     |    |            |     |     |    |     |     |
|-----|----|------------|-----|-----|----|-----|-----|
| --- | 10 | 2.5Cu      | 96  | 106 | 18 | 2.6 | 325 |
| --- | 10 | 5Cu        | 122 | 131 | 13 | 3.6 | 342 |
| --- | -- | 10Sb-2.5Cu | 129 | 136 | 8  | 2.3 | 344 |

(IODIDE Ti-BASE)

|     |    |             |     |     |    |     |     |
|-----|----|-------------|-----|-----|----|-----|-----|
| --- | 10 | 2.5Cu-1.5Fe | 117 | 132 | 11 | 2.0 | 357 |
| --- | 10 | 2.5Cu-2.5Mn | 129 | 136 | 7  | 1.9 | 331 |
| --- | 10 | 2.5Cu-4.5Mn | 139 | 149 | 10 | 1.5 | 351 |

17  
 TABLE XIV.—Continued  
 (IODIDE Ti-BASE)

| Al | Co  | Other | Tensile Properties,<br>p. s. i. $\times 1,000$ |                      | Percent<br>Elongation<br>in 1" | Min.<br>Bend, T<br>Long. | Vickers<br>Hardness |
|----|-----|-------|------------------------------------------------|----------------------|--------------------------------|--------------------------|---------------------|
|    |     |       | 0.2%<br>Offset<br>Yield                        | Ultimate<br>Strength |                                |                          |                     |
| 5  | —   |       | 24                                             | 40                   | 53                             | 0                        | 102                 |
| 5  | 1   |       | 64                                             | 78                   | 18                             | —                        | 273                 |
| 5  | 2.5 |       | 87                                             | 102                  | 6                              | —                        | 316                 |
| 5  | 1   | 0.25C | 83                                             | 103                  | 6                              | 4.5                      | 305                 |
| 5  | 2.5 | 0.25C | 113                                            | 125                  | 13                             | Br                       | 358                 |
|    |     |       | 102                                            | 125                  | 6                              | Br                       | 374                 |

(COMMERCIAL PURITY Ti-BASE)

|   |     |            |     |     |    |     |     |
|---|-----|------------|-----|-----|----|-----|-----|
| — | —   |            | 53  | 77  | 22 | 0.7 | 202 |
| 4 | 2   | 2.5 Cr     | 88  | 101 | 19 | 1.7 | 304 |
| 4 | 2   | 2.5 Cu     | 135 | 145 | 9  | 2.6 | 353 |
| 4 | 2   | 1.5 Fe     | 113 | 138 | 8  | 7.2 | 341 |
| 4 | 2   | 2.5 Mn     | 118 | 142 | 5  | Br  | 368 |
| 4 | 2   | 2.5 Mo     | 117 | 138 | 12 | 1.9 | 348 |
| 4 | 2   | 2.5 Ni     | 128 | 142 | 8  | 1.7 | 372 |
| 4 | 2   | 5Ta        | 96  | 117 | 5  | 6.2 | 296 |
| 4 | 2   | 5V         | 108 | 127 | 4  | 7.1 | 335 |
| 4 | 2   | 2.5W       | 154 | 160 | 5  | 2.3 | 368 |
| 4 | 2   | 5Cb        | 117 | 135 | 8  | 6.0 | 345 |
| — | 1   | 10Sn       | 139 | 147 | 6  | 3.8 | 353 |
| — | 2.5 | 10Sn       | 90  | 106 | 19 | 2.7 | 289 |
| — | 2.5 | 10Sn       | 108 | 125 | 11 | 2.6 | 317 |
| — | 5   | 10Sn       | 111 | 124 | 3  | Br  | 357 |
| — | 2.5 | 10Sb       | 108 | 119 | 11 | 5.4 | 309 |
| — | 2   | 10Sn-2Ni   | 97  | 118 | 12 | 4.9 | 325 |
| — | 2   | 10Sn-2.5Cu | 114 | 136 | 5  | Br  | 339 |
| — | 2   | 10Sn-2.5Mn | 147 | 153 | 9  | 4.1 | 354 |

(IODIDE Ti-BASE)

| Al | Si  |     |     |    |     |     |  |
|----|-----|-----|-----|----|-----|-----|--|
|    |     | 24  | 40  | 53 | 1.3 | 102 |  |
| —  | —   | 38  | 53  | 16 | —   | 153 |  |
| 2  | —   | 66  | 76  | 16 | —   | 273 |  |
| 2  | 1   | 72  | 93  | 16 | —   | 240 |  |
| 2  | 2   | 67  | 87  | 5  | —   | 305 |  |
| 5  | 1   | 100 | 116 | 9  | —   | 338 |  |
| 5  | 0.5 | 104 | 120 | 8  | —   | 326 |  |

(COMMERCIAL PURITY Ti-BASE)

|    |     |      |     |     |     |     |     |
|----|-----|------|-----|-----|-----|-----|-----|
| —  | 0.5 | 10Sn | 100 | 110 | 17  | 1.5 | 325 |
| —  | 1   | 10Sn | 97  | 109 | 17  | 5.0 | 330 |
| —  | 2   | 10Sn | 104 | 108 | 3   | 7.0 | 333 |
| —  | 1   | 10Sb | 97  | 108 | 15  | 2.3 | 317 |
| Al | Ni  |      |     |     |     |     |     |
| 5  | 0.5 | 76   | 90  | 13  | —   | 296 |     |
| 5  | 2.5 | 73   | 89  | 4   | —   | 318 |     |
| 5  | 5   | 87   | 106 | 5   | —   | 323 |     |
| 4  | 2   | 109  | 122 | 7   | 3.2 | 305 |     |
| 4  | 2   | 132  | 144 | 5   | 6.9 | 341 |     |
| 4  | 2   | 117  | 136 | 12  | 3.5 | 336 |     |
| 4  | 2   | 115  | 128 | 10  | 3.8 | 317 |     |
| —  | 1   | 88   | 102 | 18  | 1.8 | 283 |     |
| —  | 2.5 | 95   | 111 | 10  | 2.6 | 294 |     |
| —  | 5   | 111  | 131 | 11  | 5.7 | 327 |     |
| —  | 2.5 | 97   | 109 | 17  | 2.5 | 296 |     |
| —  | 2   | 107  | 124 | 13  | 4.0 | 342 |     |

Our researches have established that Ti-Al-Cu alloys according to the invention containing about 4 to 8% aluminum and 2 to 4% copper have excellent properties as forging alloys. A typical alloy of this type having the composition Ti-7Al-3Cu was forged at 1800° F. followed by annealing at 1800° F. and furnace cooling to randomize the structure, and was then rolled at 1700° F. to  $\frac{1}{4}$ " plate. As thus fabricated, specimens thereof were subjected to various heat treatments and their room temperature mechanical properties determined with results as shown in Table I-B supra.

As shown by the data in said table, the Ti-7Al-3Cu alloy can be heat treated by quenching from the alpha-beta field (1700° F.), or from the beta field (1840° F.). As is also shown, the greatest response to heat treatment is obtained by quenching from the beta field, which produces an increase in strength of about 35,000 p. s. i.

as compared to furnace cooling from the beta field. A better combination of strength and ductility is obtained by quenching from the alpha-beta field, where the strength is almost as high as that obtained by quenching from the beta field, and the reduction in area is above 20%. Air cooling from the alpha-beta or beta field causes a small increase in strength (about 15,000 p. s. i.), while furnace cooling from the alpha-beta field has little effect on strength. Furnace cooling from the beta field produces some loss in strength as compared with the alpha-compound, furnace-cooled condition. Quenching from the beta field and tempering to produce a random distribution of very small compound particles in an acicular alpha matrix results in an increase in strength of about 10,000 p. s. i. as compared to the alpha-compound annealed condition. The tempered alpha-beta quenched specimen does not show this strength increase, probably

because the dispersed compound particles are not randomly distributed but were present in the prior beta areas. The aging tests of said Table I-B also establish that this alloy exhibits its greatest thermal stability in the alpha-compound annealed condition (7 hours at 1400° F. and furnace cooled) either as a single treatment or as a tempering treatment following a heat treatment from above the critical.

The following Table XV shows the effect of various alpha-compound annealing cycles on the room temperature tensile properties of the Ti-7Al-3Cu alloy both prior and subsequent to aging for 100 hours at 800° F. and also after subjection to creep exposure for 100 hours at 750° F. at a stress of 65,000 p. s. i.

one employing the highest final annealing temperature (1400° F.) is the least effective from the stability standpoint. Since the other three anneals finish at lower temperatures, it appears that a gain in stability is obtained by equilibrating the alpha and compound phases at a temperature closer to the creep exposure temperature. It is to be noted from the data of this table, however, that although excellent thermal stability is obtained with the second annealing cycle listed, the stability after creep exposure is impaired with this as well as with all of the other annealing cycles.

The effect on stability of substituting various other alpha promoters, such as one or more of tin, antimony and zirconium for part or all of the aluminum in the

TABLE XV  
*Creep data and subsequent room-temperature tensile-test data of a Ti-7Al-3Cu alloy*

| Annealing Heat Treatment                                                                                                | Creep Data  |            |                        |                                |                         | Room-Temperature Tensile Properties  |           |                           |                            |
|-------------------------------------------------------------------------------------------------------------------------|-------------|------------|------------------------|--------------------------------|-------------------------|--------------------------------------|-----------|---------------------------|----------------------------|
|                                                                                                                         | Time, hours | Temp., °F. | Stress, 1,000 p. s. i. | Residual Strain, Percent in 1" | Min. Creep Rate per hr. | Tensile Properties, p. s. i. × 1,000 |           | Percent Elonga-tion in 1" | Percent Reduc-tion in Area |
|                                                                                                                         |             |            |                        |                                |                         | 0.2% Offset Yield                    | Ult. Str. |                           |                            |
| 6 hr. at 1,400° F., plus 2 hr. at 800° F., plus 24 hr. at 1,200° F., and air cool to room temp.                         | None        |            |                        |                                |                         | 125                                  | 138       | 10                        | 15                         |
| Do.                                                                                                                     | 100         | 800        | None                   |                                |                         | 132                                  | 147       | 14                        | 16                         |
| Do.                                                                                                                     | 100         | 750        | 65                     | 0.07                           | 0.0001                  | 126                                  | 131       | 3                         | 5                          |
| 6 hr. at 1,400° F., plus 24 hr. at 1,200° F., and air cool to room temp.                                                | None        |            |                        |                                |                         | 123                                  | 137       | 14                        | 23                         |
| Do.                                                                                                                     | 100         | 800        | None                   |                                |                         | 133                                  | 146       | 16                        | 16                         |
| Do.                                                                                                                     | 100         | 750        | 65                     | 0.22                           | 0.0009                  | 126                                  | 132       | 6                         | 8                          |
| 2 hr. at 1,400° F., furnace cool to 1,200° F., 4 hr. at 1,200° F., furnace cool to 1,000° F., hold 16 hr., and air cool | None        |            |                        |                                |                         | 137                                  | 147       | 6                         | 8                          |
| Do.                                                                                                                     | 100         | 800        | None                   |                                |                         | 141                                  | 150       | 8                         | 10                         |
| Do.                                                                                                                     | 100         | 750        | 65                     | 0.23                           | 0.0005                  | 136                                  | 144       | 3                         | 6                          |
| 7 hr. at 1,400° F. and furnace cool to room temp.                                                                       | None        |            |                        |                                |                         | 132                                  | 144       | 10                        | 8                          |
| Do.                                                                                                                     | 100         | 800        | None                   |                                |                         | 140                                  | 148       | 10                        | 9                          |
| Do.                                                                                                                     | 100         | 800        | 60                     | 0.247                          | 0.0009                  | (b)                                  | 100       | 2                         | 4                          |

<sup>a</sup>Transverse bar specimens.

<sup>b</sup>Brittle fracture occurred before yield.

It will be seen from the foregoing data, that of the four alpha-compound stabilizing anneals employed, the

Ti-7Al-3Cu alloy is shown by the test results in the following Table XVI:

TABLE XVI  
*Room-temperature and 1,000° F. tensile properties of alpha-dispersoid alloys*

[As annealed 7 hours at 1,400° F., furnace cooled to 1,100° F., held 16 hours at 1,100° F., and air cooled to room temperature.]

| Comp. Percent, Bal. Ti              | Exposure Data |            |                        |                        |                         | Tensile Test Data |                                      |           |                           |                      |           |
|-------------------------------------|---------------|------------|------------------------|------------------------|-------------------------|-------------------|--------------------------------------|-----------|---------------------------|----------------------|-----------|
|                                     | Time, hours   | Temp., °F. | Stress, 1,000 p. s. i. | Percent Plastic Strain | Min. Creep Rate per hr. | Test. Temp., °F.  | Tensile Properties, p. s. i. × 1,000 |           | Percent Elonga-tion in 1" | Percent Red. in Area | MBR, T, L |
|                                     |               |            |                        |                        |                         |                   | 0.2% Offset Yield                    | Ult. Str. |                           |                      |           |
| 7Al-3Cu Bar (T) <sup>1</sup>        | None          |            |                        |                        |                         | 75                | 123                                  | 137       | 14                        | 23                   |           |
|                                     | 100           | 800        | None                   |                        |                         | 75                | 133                                  | 146       | 16                        | 16                   |           |
| 7Al-3Cu Sheet (L) <sup>1</sup>      | 100           | 750        | 65                     | 0.22                   | 0.0009                  | 75                | 126                                  | 132       | 6                         | 8                    |           |
|                                     | 127           | 800        | 65                     | 0.24                   | 0.0013                  | 75                | 127                                  | 139       | 15                        | 27                   | 3.7       |
| 5Al-6Sn-3Cu Sheet (L) <sup>1</sup>  | 93            | 1,000      | 15                     | 1.32                   | 0.0128                  | 75                | 135                                  | 140       | 4                         | 10                   | 4.9       |
|                                     | None          |            |                        |                        |                         | 1,000             | 70                                   | 89        | 37                        | 63                   | 6.6       |
| 3Al-12Sn-3Cu Sheet (L) <sup>1</sup> | 78            | 800        | 65                     | 0.61                   | 0.0046                  | 75                | 139                                  | 153       | 14                        | 29                   | 4.8       |
|                                     | 75            | 1,000      | 25                     | 4.71                   | 0.0557                  | 75                | 150                                  | 161       | 12                        | 32                   | 4.0/7.0   |
| 7Al-3Cu-2Mo Sheet (L) <sup>1</sup>  | 118           | 800        | None                   |                        |                         | 75                | 152                                  | 160       | 12                        | 22                   | 8.0       |
|                                     | 99            | 800        | 70                     | 0.33                   | 0.0014                  | 75                | 148                                  | 153       | 2                         | 7                    | 10        |
|                                     | 120           | 1,000      | None                   |                        |                         | 75                | 156                                  | 159       | 1                         | 6                    |           |

TABLE XVI.—Continued

| Comp. Percent, Bal. Ti    | Exposure Data |            |                        |                        |                         | Tensile Test Data |                                             |           |                               |                      |           |
|---------------------------|---------------|------------|------------------------|------------------------|-------------------------|-------------------|---------------------------------------------|-----------|-------------------------------|----------------------|-----------|
|                           | Time, hours   | Temp., °F. | Stress, 1,000 p. s. i. | Percent Plastic Strain | Min. Creep Rate per hr. | Test. Temp., °F.  | Tensile Properties, p. s. i. $\times 1,000$ |           | Percent Elonga-<br>tion in 1" | Percent Red. in Area | MBR, T, L |
|                           |               |            |                        |                        |                         |                   | 0.2% Offset Yield                           | Ult. Str. |                               |                      |           |
| 7Al-3Cu-0.5Mo Sheet (L)   | None          |            |                        |                        |                         | 75                | 138                                         | 154       | 8                             | 9                    |           |
| 7Al-2Cu-2Mo Sheet (L)     | None          |            |                        |                        |                         | 75                | 151                                         | 164       | 4                             | 7                    |           |
| 7Al-1.5Cu-1.5Mo Sheet (L) | None          |            |                        |                        |                         | 75                | 147                                         | 159       | 13                            | 23                   |           |
| 7Al-1.5Cu-3Mo Sheet (L)   | None          |            |                        |                        |                         | 75                | 152                                         | 166       | 7                             | 11                   |           |
| 6Al-2Si-2Mo Sheet (L)     | None          |            |                        |                        |                         | 75                | 144                                         | 157       | 5                             | 10                   | 8.3       |
|                           | 118           | 800        | None                   |                        |                         | 75                | 134                                         | 145       | 10                            | 8                    |           |
|                           | 143           | 800        | 65                     | 0.10                   | 0.0004                  | 75                | 139                                         | 140       | 2                             | 3                    |           |
| 5Al-5Sn-5Zr-3Cu Bar (T)   | 2 142         | 800        | 65                     | 0.18                   | 0.0012                  | 75                | 147                                         | 148       | 2                             | 1                    |           |
|                           | 120           | 1,000      | None                   |                        |                         | 75                | 143                                         | 143       | 0                             | 0                    |           |
|                           | None          |            |                        |                        |                         | 1,000             | 84                                          | 109       | 18                            | 22                   |           |
|                           | None          |            |                        |                        |                         | 75                | 128                                         | 139       | 14                            | 17                   |           |
|                           | 118           | 800        | None                   |                        |                         | 75                | 137                                         | 143       | 4                             | 8                    |           |
| 6Al-6Zr-3Cu Bar (T)       | 117           | 800        | 65                     | 0.153                  | 0.0003                  | 75                | 136                                         | 136       | 0                             | 0                    |           |
|                           | 120           | 1,000      | None                   |                        |                         | 75                | 139                                         | 149       | 12                            | 16                   |           |
|                           | 99            | 800        | 65                     | 0.167                  | 0.0014                  | 75                | 123                                         | 123       | 1                             | 3                    |           |
|                           | 98            | 1,000      | 15                     | 0.130                  | 0.0012                  | 75                | 141                                         | 154       | 14                            | 12                   |           |
|                           | None          |            |                        |                        |                         | 75                | 123                                         | 123       | 12                            | 13                   |           |
|                           | 118           | 800        | None                   |                        |                         | 75                | 129                                         | 135       | 12                            | 7                    |           |
| 4Al-12Zr-3Cu Bar (T)      | 139           | 800        | 65                     | 0.18                   | 0.0005                  | 75                | 127                                         | 130       | 9                             | 8                    |           |
|                           | 115           | 1,000      | 15                     | 0.25                   | 0.0016                  | 75                | 123                                         | 130       | 14                            | 11                   |           |
|                           | 97            | 1,000      | 15                     | 0.20                   | 0.0003                  | 75                | 115                                         | 126       | 2                             | 4                    |           |
|                           | None          |            |                        |                        |                         | 1,000             | 78                                          | 91        | 34                            | 69                   |           |
|                           | None          |            |                        |                        |                         | 75                | 134                                         | 142       | 14                            | 20                   |           |
|                           | 104           | 800        | 70                     | 0.06                   | 0.0003                  | 75                | 137                                         | 146       | 7                             | 15                   |           |
| 4Al-12Zr-3Cu Bar (T)      | 98            | 800        | 65                     | 0.09                   | 0.0008                  | 75                | 137                                         | 145       | 10                            | 18                   |           |
|                           | 104           | 1,000      | 10                     | 0.10                   | 0.0005                  | 75                | 135                                         | 141       | 9                             | 18                   |           |
|                           | 99            | 1,000      | 15                     | 0.19                   | 0.0012                  | 75                | 134                                         | 144       | 20                            | 53                   |           |
|                           | None          |            |                        |                        |                         | 800               | 88                                          | 107       | 16                            | 53                   |           |
|                           | 118           | 800        | None                   |                        |                         | 75                | 128                                         | 139       | 14                            | 17                   |           |
| 6Al-6Zr-3Cu Bar (T)       | 117           | 800        | 65                     | 0.15                   | 0.0003                  | 75                | 137                                         | 143       | 4                             | 8                    |           |
|                           | 2 144         | 800        | 65                     | 0.16                   | Nil                     | 75                | 136                                         | 150       | 0                             | 0                    |           |
|                           | 120           | 1,000      | None                   |                        |                         | 75                | 139                                         | 149       | 5                             | 7                    |           |
|                           | None          |            |                        |                        |                         | 1,000             | 82                                          | 105       | 26                            | 64                   |           |
|                           | None          |            |                        |                        |                         | 75                | 91                                          | 102       | 18                            | 40                   |           |
| 4Al-3Cu Sheet (L)         | 142           | 800        | 50                     | 4.49                   | 0.0238                  | 75                | 80                                          | 92        | 11                            | 36                   |           |
|                           | 25            | 800        | 65                     | 32.20                  | 0.3750                  | 75                | 111                                         | 114       | 10                            | 21                   |           |
|                           | 74            | 1,000      | 10                     | 1.28                   | 0.0163                  | 75                | 75                                          | 74        | 21                            | 35                   | 2.5       |
| 2Al-3Cu Sheet (L)         | None          |            |                        |                        |                         | 75                | 63                                          | 78        | 18                            | 44                   | 2.1       |
|                           | 0.1           | 800        | 50                     | 17.10                  |                         | 75                | 108                                         | 124       | 14                            | 33                   | 2.3       |
|                           | 0.1           | 800        | 55                     | 20.00                  |                         | 75                | 114                                         | 123       | 12                            | 28                   |           |
|                           | 79            | 1,000      | 10                     | 2.11                   | 0.0253                  | 75                | 110                                         | 125       | 11                            | 32                   | 2.6       |
| 12Sn-3Cu Sheet (L)        | None          |            |                        |                        |                         | 75                | 97                                          | 110       | 17                            | 25                   | 2.6       |
|                           | 96            | 800        | 50                     | 0.83                   | 0.0076                  | 75                | 106                                         | 118       | 10                            | 19                   | 2.9       |
|                           | 99            | 1,000      | 10                     | 0.63                   | 0.0048                  | 75                | 100                                         | 112       | 10                            | 23                   | 2.1       |
| 12Sb-3Cu Sheet (L)        | None          |            |                        |                        |                         | 75                | 62                                          | 79        | 27                            | 43                   | 2.7       |
|                           | 102           | 800        | 50                     | 0.13                   | 0.0017                  | 75                | 72                                          | 83        | 17                            | 39                   | 3.2       |
|                           | 136           | 1,000      | 15                     | 0.56                   | 0.0052                  | 75                | 65                                          | 85        | 16                            | 39                   | 2.4       |
| 3Cu Sheet (L)             | None          |            |                        |                        |                         | 75                | 147                                         | 157       | 7                             | 8                    | 1.9       |
|                           | 96            | 800        | 30                     | 1.44                   | 0.0104                  | 75                | 150                                         | 162       | 12                            | 21                   |           |
|                           | 96            | 1,000      | 5                      | 0.60                   | 0.0031                  | 75                | 151                                         | 161       | 10                            | 23                   |           |
| 5Al-12Zr-6Cu Bar (L)      | None          |            |                        |                        |                         | 75                | 96                                          | 121       | 24                            | 57                   |           |
|                           | 97            | 800        | 65                     | 0.079                  | Nil                     | 75                | 151                                         | 162       | 7                             | 9                    |           |
| Bar (T)                   | 98            | 1,000      | 25                     | 0.436                  | 0.0038                  | 75                | 150                                         | 159       | 12                            | 10                   |           |
|                           | 69            | 1,000      | 15                     | 0.056                  | 0.0016                  | 75                | 146                                         | 156       | 10                            | 23                   |           |
|                           | 99            | 800        | 75                     | 0.105                  | 0.0060                  | 75                | 151                                         | 161       | 10                            | 10                   |           |
| Bar (L)                   |               |            |                        |                        |                         | 800               | 96                                          | 108       | 28                            | 60                   |           |
|                           |               |            |                        |                        |                         | 1,000             | 90                                          | 108       | 28                            | 60                   |           |

<sup>1</sup> Type Specimen.<sup>2</sup> 120 hrs. at 1,000° F. stabilization anneal prior to creep exposure.<sup>3</sup> Average properties of 7, 1/2 lb. ingots.

In the data shown by the above tests, three levels of alpha stabilizer additions were made to the Ti-3Cu alloy. Tin and antimony were substituted for part or all of the aluminum in the 3:1 ratio above mentioned. In other alloys shown by the data, zirconium is added in varying amounts as an alpha promoter, while in still other data, molybdenum was added as a beta-isomorphous promoter.

The data given in the above table shows that the substitution of tin for part of the aluminum at the 7% (equivalent) aluminum level does not impart greater stability. Higher strength is obtainable with higher tin-to-aluminum ratio, but the stability remains about the same. At the 4% (equivalent) aluminum level, the Ti-12Sn-3Cu and the Ti-12Sb-3Cu alloys are stronger than the Ti-4Al-3Cu composition. More-

over, the Ti-12Sn-3Cu is almost completely stable. Also both the Ti-4Al-3Cu and Ti-12Sb-3Cu alloys are more stable than the alloys containing higher alpha stabilizer additions. The two alloys with no or low alpha stabilizer additions (Ti-3Cu and Ti-2Al-3Cu) also show high degrees of stability, as shown particularly by the bend ductility values. The addition of 2% molybdenum imparts high strength with adequate ductility, but the resulting alloys are unstable.

A comparison of the elongation data given in the above table suggests that two different types of embrittlement are encountered in these alloys. The first, due to copper precipitation, is not too serious, resulting in only slight loss in ductility. Embrittlement of this type is seen quite clearly in compositions such as Ti-3Cu, Ti-4Al-3Cu, Ti-12Sn-3Cu, etc. The loss in ductil-

ity is about equally great at 800 and 1000° F. The second type of embrittlement is believed to be due to ordering in the alpha solid solution. The greater the amount of aluminum plus tin and/or antimony, the greater the tendency toward ordering. No embrittlement from this action is encountered when the aluminum equivalent ( $Al+Sn, Sb/3$ ) is less than about 6 weight percent (roughly 10 atomic percent). Embrittlement is observed first at 800° F., then, as more aluminum plus tin is added, 10 at 1000° F. Thus,  $Ti-7Al-3Cu$ ,  $Ti-5Al-6Sn-3Cu$ , and  $Ti-3Al-12Sn-3Cu$  show marked embrittlement at 800° F., but none at 1000° F. The addition of 2% molybdenum evidently increases the tendency toward embrittlement, as shown by the tendency for  $Ti-7Al-2Mo-3Cu$  to be embrittled both at 800 and 1000° F. Presumably the detrimental effect of molybdenum is connected with precipitation of  $Ti_2Cu$ .

The replacement of aluminum plus tin and/or antimony by zirconium is effective in removing the tendency toward ordering. For example,  $Ti-5Al-5Sn-5Zr-3Cu$  (6% aluminum equivalent) is extremely unstable,  $Ti-6Al-6Zr-3Cu$  (6% aluminum equivalent) is unstable at 800° F. only, and  $Ti-4Al-12Zr-3Cu$  (4% aluminum equivalent) is stable. Also, since  $Ti-7Al-3Cu$  was embrittled only at 800° F., it is apparent that zirconium additions lower the permissible aluminum-plus-tin and/or antimony content slightly, possibly as much as 1% aluminum equivalent.

Alloys according to the invention containing about 5 to 8% copper and 8 to 14% tin and preferably about 6 to 7% copper and 10% tin have excellent properties for use in sheet form, i. e., in the airplane industry for wing coverings and the like. As alpha-compound annealed at about 1475° F., these alloys are relatively soft, have relatively low yield strength and excellent bend ductility and thus can be easily formed and bent to shape. In addition, they undergo a marked strengthening and hardening when subjected to relatively slow cooling from temperature above the beta-transus, i. e., from about 1500-1550° F. or above. The fact that these alloys can be strengthened by this relatively simple and short-time heat treatment consisting in slow air cooling from above the critical is of great practical advantage, because it permits the use of jigs to hold the fabricated parts in position, such as a wing foil and air frame, during the strengthening heat treatment. This relatively short-time heat treatment required for strengthening these alloys, stands in marked contrast to the long periods of heat treatment required for alloys which are hardened and strengthened by the age-hardening procedure. These  $Ti-Sn-Cu$  alloys also possess the further advantage that after being strengthened by the air cooling heat treatment aforesaid, they may be thermally stabilized by a relatively simple tempering treatment in air at about 1000-1100° F. with considerable leeway permitted in both time and temperature of such treatment.

The air hardening characteristics of these alloys is well illustrated by resort to the Jominy test according to which a bar of the alloy is heated above critical, for example, at 1540° F., and thereupon end-quenched in water. The results of such a test carried out on a  $Ti-10Sn-7Cu$  alloy are shown in Figure 1 of the annexed drawings by the graph marked "as quenched." In this drawing, the distance from the quenched end in inches is plotted as abscissae while the Vickers hardness of the quenched specimen at any given distance from the quenched end is plotted as ordinates. The important features of this end-quenched graph as thus depicted are: (1) the alloy is soft in the quenched condition, (2) the peak hardness occurs at a distance of about  $\frac{1}{2}$ " from the quenched end, thus

being equivalent to a cooling rate of about 10-15 seconds to cool from 1540° F. down to 1000° F. (30-50° F. per second), (3) even with very slow cooling rates, as depicted at greater distances from the quenched end, appreciable hardening occurs.

The low as-quenched hardness is indicative of either soft martensite formation or soft retained beta, or both. Although the structure at the quenched end appears to be chiefly martensite, it is probable that some retained beta is present also. The structure at the peak hardness is predominantly martensite with about 5% eutectoid structure (some omega-harden beta also may be present which cannot be seen in the structure). A complete eutectoid structure is not obtained until about 2" from the quenched end.

To check the stability and the effect of tempering on the various structures above referred to, additional specimens were end-quenched and were re-heated for 16 hours at 800, 1000, 1100 and 1200° F., respectively, and tested for hardness with results also as shown in Figure 1 by the graphs, respectively, so designated. It is evident from these additional tests that the martensitic structure near the quenched end is not stable. Thus, as shown in this drawing, aging at 800° F. causes an increase in hardness even above the peak hardness to a distance of about 1" from the quenched end. Beyond this distance, where the structure is predominantly eutectoid, there is no significant change in hardness. Tempering for 16 hours at 1000° F. causes a decrease in hardness throughout the peak hardness range, giving a fairly uniform hardness along the length of the specimen. Similarly, tempering at 1200° F. causes a softening over the entire length of the specimen to a substantially uniform hardness. These data show that in order to obtain a stable structure, a low enough cooling rate should be used to secure a eutectoid structure; and also that it is possible to temper the high-hardness martensitic structure to a hardness about the same as the eutectoid structure.

It has heretofore been shown in U. S. Patent 2,769,707 to M. B. Vordahl, that tin slows down the beta decomposition reaction rates in alpha-beta, Ti-base alloys. Our investigations indicate that tin acts similarly in titanium-copper alloys, as evidenced by the Jominy end-quench tests shown in Figures 2 and 3 of the accompanying drawings, Figure 2 illustrating the effect on hardenability of varying the tin content at the  $Ti-7Cu$  level, and Figure 3 illustrating the effect of varying the copper content on hardenability of the  $Ti-10Sn$  base alloy. It will be seen from these graphs that maximum depth of hardening occurs at the 7% copper (eutectoid) level. The shallower depth of hardening which occurs with both hypo- and hyper-eutectoid alloys is believed to be caused by proeutectoid alpha or compound particles acting as nucleation sites for the eutectoid reaction. It is apparent from these graphs that to obtain maximum depth of hardening, the copper content should be of the eutectoid (7%) composition and the tin content should be kept as high as possible.

Referring to Figure 2, it will be seen that as the tin content is decreased, the hardness peak shifts progressively toward the quenched end, so that these  $Ti-Sn-Cu$  alloys containing about 6% and under of tin, obtain their maximum hardness on quenching from above the critical. Conversely, the fact that the hardness peak shifts progressively further from the quenched end as the tin content is increased, evidences the fact above mentioned that the tin addition is slowing down the beta decomposition reaction rate.

The  $Ti-10Sn-7Cu$  alloy is relatively soft in the alpha-compound annealed condition and is capable of being

hardened by air-hardening treatment to useful strength levels. Typical tensile properties of this alloy in the alpha-compound annealed condition are:

|                                      |          |
|--------------------------------------|----------|
| 0.2% offset yield strength, p. s. i. | 110,000  |
| Ultimate strength, p. s. i.          | 120,000  |
| Elongation, percent in 1 inch        | 10       |
| Reduction in area, percent           | 30       |
| Minimum bend radius, T               | 1.5 to 2 |

The effect on tensile properties of heat treating this alloy from above the critical is dependent upon the solution-annealing temperature and upon the cooling rate, as shown by the data in the following Table XVII:

The beta-transus for this alloy occurs at about 1500° F. and it will be seen from the data in the above table that the maximum strength is imparted to the alloy when it is cooled from the heat treating temperature to below 1000° F. in about ten seconds. It was indicated above by the end-quench graphs shown in Figure 1, that tempering for 16 hours at 1000° F. tends to overcome the hardness variations caused by the different cooling rates incorporated in the end-quench tests. Also variations in tensile properties tend to be smoothed out by tempering treatments.

In the alpha-compound annealed condition, the stability of the Ti-10Sn-7Cu alloy is good in both unstressed and stressed conditions as shown by the data in Table XVIII:

TABLE XVIII

*Tensile test results on a Ti-10Sn-7Cu alloy before and after aging and creep exposure*

| Annealing Heat Treatment                                                                                                        | TTSS Exposure |           |                        |                                | Tensile Properties, p. s. i. $\times 1,000$ |           | Percent Elongation in 1" | Percent Reduction in Area |
|---------------------------------------------------------------------------------------------------------------------------------|---------------|-----------|------------------------|--------------------------------|---------------------------------------------|-----------|--------------------------|---------------------------|
|                                                                                                                                 | Time, hours   | Temp, °F. | Stress, 1,000 p. s. i. | Residual Strain, Percent in 1" | 0.2% Offset Yield                           | Ult. Str. |                          |                           |
| 6 hr. at 1,400° F. plus 2 hr. at 800° F., plus 24 hr. at 1,200° F., and air cool                                                | None          |           |                        |                                | 100                                         | 111       | 14                       | 23                        |
|                                                                                                                                 | 100           | 800       | None                   | 1.61                           | 99                                          | 106       | 8                        | 37                        |
| 6 hr. at 1,400° F. plus 24 hr. at 1,200° F., and air cool                                                                       | 100           | 750       | 65                     |                                | 110                                         | 116       | 11                       | 20                        |
|                                                                                                                                 | 100           | 800       | None                   |                                | 100                                         | 110       | 12                       | 30                        |
| 2 hr. at 1,400° F., furnace cool to 1,200° F., 4 hr. at 1,200° F., furnace cool to 1,000° F., 16 hr. at 1,000° F., and air cool | 100           | 750       | 65                     | b 3.04                         | 102                                         | 110       | 11                       | 25                        |
|                                                                                                                                 | 100           | 800       | None                   |                                | 110                                         | 113       | 4                        | 17                        |
| 16 hr. at 1,400° F. and air cool                                                                                                | None          |           |                        |                                | 100                                         | 109       | 10                       | 29                        |
|                                                                                                                                 | 100           | 800       | None                   | 1.64                           | 106                                         | 116       | 13                       | 21                        |
| Do                                                                                                                              | 100           | 750       | 65                     |                                | 111                                         | 116       | 9                        | 19                        |
|                                                                                                                                 | 100           | 800       | None                   |                                | 109                                         | 126       | 10                       | 24                        |
| Do                                                                                                                              | 100           | 750       | 65                     | c 0.55                         | 111                                         | 124       | 12                       | 30                        |
|                                                                                                                                 | 100           | 800       | None                   |                                | 120                                         | 124       | 4                        | 15                        |

a 0.00357 percent per hour minimum creep rate during TTSS exposure.

b 0.0142 percent per hour minimum creep rate during TTSS exposure.

c 0.00316 percent per hour minimum creep rate during TTSS exposure.

d 0.00166 percent per hour minimum creep rate during TTSS exposure.

TABLE XVII

*Tensile properties of Ti-10Sn-7Cu alloy in several heat-treated conditions*

| Heat Treatment                | Tensile Properties, p. s. i. $\times 1,000$ |                            |                   | Percent Elonga-tion in 1" | Percent Reduc-tion in Area |
|-------------------------------|---------------------------------------------|----------------------------|-------------------|---------------------------|----------------------------|
|                               | Cooling Rate, °F. sec.                      | 0.2% Offset Yield Strength | Ultimate Strength |                           |                            |
| Solution Annealing Temp., °F. |                                             |                            |                   |                           |                            |
| 1,500                         | 50                                          | 130                        | 142               | 6                         | 13                         |
| 1,500                         | 50                                          | 129                        | 142               | 7                         | 27                         |
| 1,525                         | 50                                          | 142                        | 155               | 5                         | 17                         |
| 1,525                         | 50                                          | 137                        | 153               | 7                         | 18                         |
| 1,540                         | 2                                           | 92                         | 166               | 8                         | 9                          |
| 1,540                         | 2                                           | 98                         | 162               | 8                         | 8                          |
| 1,540                         | 10                                          | 202                        | 214               | 2                         | 8                          |
| 1,540                         | 10                                          | 191                        | 202               | 1                         | 5                          |
| 1,540                         | 10                                          | 183                        | 192               | 1                         | 8                          |
| 1,540                         | 50                                          | 154                        | 168               | 3                         | 8                          |
| 1,540                         | 50                                          | 158                        | 171               | 2                         | 2                          |
| 1,540                         | 50                                          | 158                        | 170               | 2                         | 2                          |
| 1,540                         | 50                                          | 154                        | 168               | 3                         | 8                          |
| 1,540                         | 100                                         | 157                        | 168               | 2                         | 5                          |
| 1,550                         | 2                                           | 112                        | 174               | 8                         | 15                         |
| 1,550                         | 50                                          | 177                        | 189               | 2                         | 14                         |
| 1,550                         | 50                                          | 168                        | 175               | 3                         | 14                         |
| 1,550                         | 50                                          | 167                        | 185               | 3                         | 7                          |

\* Time to cool from heat-treating temperature to below 1,000° F.

Although the uniform elongation of this alloy in the annealed condition is only about 2% at room temperature, it is increased to about 10% on heating to the relatively low temperature of 200° F., thereby to permit an excellent stretch forming.

As pointed out in U. S. Patent 2,669,514 to Finlay et al., tin in excess of about 5%, imparts to Ti-base alloys, excellent contamination resistance to atmospheric gases at elevated temperatures. This is true of the Ti-10Sn-7Cu alloy, which, in addition, has excellent oxidation resistance at the solution-annealing temperature of 1525° F. and at the annealing temperature of 1400° F. Less than 0.025 mil of the metal is lost in two hours at 1525° F. and only about 0.03 mil is lost in sixteen hours at 1400° F. In terms of metal loss per year, this amounts to about 0.015" per year at 1400° F. and 0.075" per year at 1525° F.

The effect on room temperature and tensile properties of varying the tin and copper contents of these Ti-Sn-Cu sheet alloys, in both the alpha-compound annealed and heat treated conditions, is shown in the following Table XIX. The succeeding Table XX shows corresponding data for the Ti-10Sn-4Cu-2Fe and

75 Ti-12Sn-5Cu-2Mo alloys.

TABLE XIX

*Room-temperature tensile test properties of various heat-treatable alpha-dispersoid sheet alloys*

[Alpha-compound annealed plus solution heat treat as indicated.]

## Ti-8Sn-7Cu

| Heat Treatment (20 Minutes at Temperature)             | VHN<br>(Surface) | Tensile Properties,<br>p. s. i. $\times 1,000$ |                      | Percent<br>Elonga-<br>tion in<br>1" | Percent<br>Reduc-<br>tion in<br>Area |
|--------------------------------------------------------|------------------|------------------------------------------------|----------------------|-------------------------------------|--------------------------------------|
|                                                        |                  | 0.2%<br>Offset<br>Yield                        | Ultimate<br>Strength |                                     |                                      |
| None <sup>a</sup>                                      | 265              | 104                                            | 114                  | 13                                  | 31                                   |
| None <sup>a</sup>                                      | 275              | 111                                            | 119                  | 10                                  | 28                                   |
| 1,500° F., slow air cool                               | 328              | 139                                            | 152                  | 5                                   | 15                                   |
| 1,525° F., water quench                                | 320              | 91                                             | 152                  | 6                                   | 12                                   |
| 1,525° F., water quench plus temper <sup>b</sup>       | 370              | 145                                            | 159                  | 1                                   | 7                                    |
| 1,525° F., fast air cool                               | 445              |                                                | 189                  | 1                                   | 6                                    |
| 1,525° F., fast air cool plus temper <sup>b</sup>      | 390              | 168                                            | 175                  | 1                                   | 10                                   |
| 1,525° F., slow air cool                               | 360              | 162                                            | 173                  | 1                                   | 10                                   |
| 1,525° F., slow air cool plus temper <sup>b</sup>      | 385              | 170                                            | 177                  | 1                                   | 8                                    |
| 1,525° F., very slow air cool                          | 380              | 147                                            | 162                  | 3                                   | 10                                   |
| 1,525° F., very slow air cool plus temper <sup>b</sup> | 330              | 142                                            | 156                  | 3                                   | 11                                   |
| 1,550° F., slow air cool                               | 395              | 184                                            | 195                  | 1                                   | 8                                    |

## Ti-10Sn-7Cu

|                          |     |     |     |   |    |
|--------------------------|-----|-----|-----|---|----|
| 1,550° F., slow air cool | 324 | 129 | 142 | 7 | 27 |
| Duplicate specimen       | 326 | 130 | 142 | 6 | 13 |
| 1,525° F., slow air cool | 336 | 142 | 155 | 5 | 17 |
| Duplicate specimen       | 329 | 137 | 153 | 7 | 18 |
| 1,550° F., slow air cool | 386 | 168 | 175 | 3 | 14 |
| Duplicate specimen       | 396 | 167 | 185 | 3 | 7  |

## Ti-11Sn-6Cu

|                                                     |     |     |     |    |    |
|-----------------------------------------------------|-----|-----|-----|----|----|
| None <sup>a</sup>                                   | 290 | 112 | 122 | 11 | 32 |
| 1,525° F., slow air cool <sup>c</sup>               | 416 |     | 106 |    |    |
| 1,525° F., slow air cool plus temper <sup>b,c</sup> | 403 |     | 149 |    |    |

## Ti-12Sn-5Cu

|                                                        |     |     |     |    |    |
|--------------------------------------------------------|-----|-----|-----|----|----|
| None <sup>a</sup>                                      | 285 | 106 | 118 | 11 | 33 |
| None <sup>a</sup>                                      | 295 | 105 | 119 | 11 | 29 |
| 1,500° F., slow air cool                               | 340 | 143 | 154 | 4  | 22 |
| 1,525° F., water quench                                | 345 | 108 | 159 | 7  | 32 |
| 1,525° F., water quench plus temper <sup>b</sup>       | 400 | 162 | 168 | 1  | 4  |
| 1,525° F., fast air cool                               | 390 | 169 | 186 | 2  | 13 |
| 1,525° F., fast air cool plus temper <sup>b</sup>      | 370 | 153 | 165 | 3  | 5  |
| 1,525° F., slow air cool                               | 365 | 157 | 168 | 3  | 11 |
| 1,525° F., slow air cool plus temper <sup>b</sup>      | 370 | 146 | 157 | 3  | 11 |
| 1,525° F., very slow air cool                          | 340 | 135 | 147 | 6  | 15 |
| 1,525° F., very slow air cool plus temper <sup>b</sup> | 345 | 138 | 150 | 5  | 11 |
| 1,550° F., slow air cool                               | 375 | 177 | 191 | 3  | 8  |

## Ti-12Sn-4Cu

|                     |     |    |     |    |    |
|---------------------|-----|----|-----|----|----|
| None <sup>(a)</sup> | 294 | 94 | 109 | 11 | 24 |
|---------------------|-----|----|-----|----|----|

## Ti-12Sn-3Cu

|                                                                            |     |    |     |    |    |
|----------------------------------------------------------------------------|-----|----|-----|----|----|
| None <sup>(a)</sup>                                                        | 295 | 94 | 110 | 11 | 28 |
| 1,300° F., furnace cool to 1,000° F., hold 1 hr. at 1,000° F. and air cool | 310 | 95 | 106 | 14 | 30 |

## Ti-14Sn-5Cu

|                     |       |  |  |  |  |
|---------------------|-------|--|--|--|--|
| None <sup>(a)</sup> | d 362 |  |  |  |  |
|---------------------|-------|--|--|--|--|

## Ti-14Sn-3Cu

|                     |     |     |     |   |    |
|---------------------|-----|-----|-----|---|----|
| None <sup>(a)</sup> | 337 | 124 | 136 | 3 | 14 |
|---------------------|-----|-----|-----|---|----|

(a) Alpha-plus-compound annealed 16 hrs. at 1,400° F. and air cooled.

(b) Tempered 2 hrs. at 1,100° F. and air cooled.

(c) Brittle fracture occurring in shoulder area.

(d) Longitudinal MBR,  $T=10$ .

(e) Longitudinal MBR,  $T=2.9/6.5$ .

TABLE XX

Room temperature tensile test properties of Ti-10Sn-4Cu-2Fe and  
Ti-12Sn-5Cu-2Mo alloys

## TI-10Sn-4Cu-2Fe

| Heat Treatment |               |                    | Tensile Properties,<br>p. s. i. $\times 1,000$ |                      | Percent<br>Elongation<br>in 1" | Percent<br>Reduction<br>in Area | VHN |
|----------------|---------------|--------------------|------------------------------------------------|----------------------|--------------------------------|---------------------------------|-----|
| Time, hours    | Temp.,<br>°F. | Cooling Rate       | 0.2%<br>Offset<br>Yield                        | Ultimate<br>Strength |                                |                                 |     |
| 7              | 1,200         | Fast air cool..... | 116                                            | 125                  | 7                              | 29                              | 315 |
| 7/8            | 1,280         | Slow air cool..... | 124                                            | 136                  | 10                             | 15                              | 312 |
| 1/2            | 1,360         | .....do.....       | 114                                            | 128                  | 4                              | 19                              | 317 |
| 7/8            | 1,400         | .....do.....       | 129                                            | 161                  | 5                              | 12                              | 362 |
| 7/8            | 1,460         | .....do.....       | 184                                            | 185                  | 1                              | 6                               | 445 |

## TI-12Sn-5Cu-2Mo

|     |       |                         |     |     |    |     |     |
|-----|-------|-------------------------|-----|-----|----|-----|-----|
| 16  | 1,400 | Fast air cool.....      | 81  | 138 | 10 | 19  | 280 |
| 16  | 1,400 | .....do.....            | 82  | 138 | 10 | 26  | 280 |
| 7/8 | 1,500 | Slow air cool.....      | 129 | 132 | 1  | 1   | 354 |
| 7/8 | 1,525 | Quench.....             | 60  | 157 | 13 | 27  | 318 |
| 7/8 | 1,525 | Fast air cool.....      | 58  | 165 | 13 | 24  | 295 |
| 7/8 | 1,525 | Slow air cool.....      | 127 | 147 | 3  | 8   | 361 |
| 7/8 | 1,525 | Very slow air cool..... | 167 | 170 | 1  | 6   | 484 |
| 7/8 | 1,550 | Slow air cool.....      | 143 | 168 | 1  | 6   | 400 |
| 7/8 | 1,525 | Quench.....             | 177 | 1   | 3  | 488 | 475 |
| 7/8 | 1,525 | Fast air cool.....      | 172 | 1   | 5  | 475 | 470 |
| 7/8 | 1,525 | Slow air cool.....      | 186 | 1   | 3  | 470 | 448 |
| 7/8 | 1,525 | Very slow air cool..... | 176 | 178 | 1  | 6   | 448 |

<sup>a</sup> Tempered 2 hrs. at 1,100° F. after heat treatment indicated.

The above tables show that the substitution of 2% iron for part of the copper lowers the permissible solution annealing temperature. However, our further tests have shown that substitution of 4% iron for part of the copper produces an alloy which is not responsive to heat treatment on slow air cooling. Substitution of 2% iron lowers the effective solution-annealing temperature by about 75-100° F., and lowers the eutectoid temperature by about 200-250° F. The above data also shows that substitution of molybdenum for part of the copper as a sluggish beta stabilizer to slow down the beta decomposition reaction, is quite effective in this respect. As shown, molybdenum also stabilizes the beta phase sufficiently so that, in the quenched and fast air cooled conditions, the alloy is mechanically unstable as evidenced by low yield strength and by the high ultimate to yield strength ratio.

The alloys of the invention may be produced by arc melting in an inert atmosphere, such as argon, in a cold mold furnace, for example, one employing a water-cooled crucible, or by equivalent procedures which substantially prevent atmospheric contamination or contamination by other elements productive of undue embrittlement or impairment of properties.

These alloys are useful in sheet form with minimum bend ductilities as high as 20T, and may be forged or rolled with tensile elongations as low as 1 or 2%.

Even in the fully annealed condition, the majority of these alloys have tensile strengths at room temperature of at least 100,000 p. s. i.; while those that do not may be heat treated as by quenching from the beta or alpha-beta fields to impart thereto a tensile strength of at least 100,000 p. s. i.

This application is a continuation-in-part of our pending applications as follows: Serial No. 515,539, filed June 14, 1955 (now abandoned), and Serial No. 421,980, filed April 8, 1954 (now abandoned), which in turn is a continuation-in-part of our now abandoned case Serial No. 270,896, filed February 9, 1952; and Serial Nos. 393,578, filed November 23, 1953 (now U. S. Patent 2,796,347, granted June 18, 1957); 396,756, filed December 7, 1953 (now U. S. Patent 2,797,996, granted July 2, 1957); 384,326, filed October 5, 1953 (now aban-

doned); 392,492, filed November 16, 1953, now abandoned.

35 What is claimed is:

1. An alloy consisting essentially of about: 0.5 to 23% of at least one alpha promoter selected from the group consisting of aluminum, tin, antimony and zirconium, but not to exceed 12% aluminum and 19% antimony, 0.5 to 20% of at least one active eutectoid beta promoter selected from the group consisting of copper, nickel, cobalt, silicon and beryllium, but not to exceed 12% of nickel and cobalt, 3% of silicon and 2% of beryllium, balance substantially titanium, characterized in being materially hardened and strengthened on heating above the critical temperature, until a beta-containing microstructure is obtained and thereupon rapidly cooling to a temperature substantially below the critical.
2. An alloy consisting essentially of about: 0.5 to 23% of at least one alpha promoter selected from the group consisting of aluminum, tin, antimony and zirconium, but not to exceed 12% aluminum and 19% antimony, 0.5 to 20% of at least one active eutectoid beta promoter selected from the group consisting of copper, nickel, cobalt, silicon and beryllium, but not to exceed 12% of nickel and cobalt, 3% of silicon and 2% of beryllium, up to 0.5% of elements of the group carbon, oxygen and nitrogen, but not to exceed 0.4% oxygen and 0.25% nitrogen, balance substantially titanium, characterized in having in the annealed condition a tensile strength of at least 100,000 p. s. i. and a minimum tensile elongation of about 2% and in being materially hardened and strengthened on heating above the critical temperature, until a beta-containing microstructure is obtained and thereupon rapidly cooling to a temperature substantially below the critical.
3. An alloy consisting essentially of about: 0.5 to 23% of at least one alpha promoter selected from the group consisting of aluminum, tin, antimony and zirconium, but not to exceed 12% aluminum and 19% antimony, 0.5 to 20% of copper, and the balance substantially titanium, characterized in having in the annealed condition a tensile strength of at least 100,000 p. s. i., a minimum tensile elongation of about 2%, and in being ma-

70  
75

terially hardened and strengthened on heating above the critical temperature until a beta-containing microstructure is obtained and thereupon rapidly cooling to a temperature substantially below the critical.

4. An alloy consisting essentially of about: 0.5 to 23% of at least one alpha promoter selected from the group consisting of aluminum, tin, antimony and zirconium, but not to exceed 12% aluminum and 19% antimony, 0.5 to 12% of at least one active eutectoid beta promoter selected from the group consisting of nickel and cobalt, and the balance substantially titanium, characterized in having in the annealed condition a tensile strength of at least 100,000 p. s. i., a minimum tensile elongation of about 2%, and in being materially hardened and strengthened on heating above the critical temperature, until a beta-containing microstructure is obtained and thereupon rapidly cooling to a temperature substantially below the critical.

5. An alloy consisting essentially of about: 0.5 to 23% of at least one alpha promoter selected from the group consisting of aluminum, tin, antimony and zirconium, but not to exceed 12% aluminum and 19% antimony, 0.5 to 3% of the active eutectoid beta promoter silicon, and the balance substantially titanium, characterized in having in the annealed condition a tensile strength of at least 100,000 p. s. i., a minimum tensile elongation of about 2%, and in being materially hardened and strengthened on heating above the critical temperature, until a beta-containing microstructure is obtained and thereupon rapidly cooling to a temperature substantially below the critical.

6. An alloy consisting essentially of about: 0.5 to 23% of at least one alpha promoter selected from the group consisting of aluminum, tin, antimony and zirconium, but not to exceed 12% aluminum and 19% antimony, 0.1 to 2% of the active eutectoid beta promoter beryllium, and the balance substantially titanium, characterized in having in the annealed condition a tensile strength of at least 100,000 p. s. i., a minimum tensile elongation of about 2%, and in being materially hardened and strengthened on heating above the critical temperature, until a beta-containing microstructure is obtained and thereupon rapidly cooling to a temperature substantially below the critical.

7. An alloy consisting essentially of about: 0.5 to 20% of at least one active eutectoid beta promoter selected from the group consisting of copper, nickel, cobalt and beryllium, but not to exceed 12% nickel and cobalt, 3% silicon and 2% beryllium, said alloy also containing at least one alpha promoter selected from the group consisting of aluminum, tin and antimony in total amount such that the sum of aluminum plus one-third the tin plus one-third the antimony is under 6% by weight of the total alloy, said alloy also containing about 1 to 20% zirconium, balance substantially titanium, characterized in being materially hardened and strengthened on heating above the critical temperature until a beta-containing microstructure is obtained, and thereupon rapidly cooling to a temperature substantially above the critical, said alloy being also characterized by high stability after exposure in both stressed and unstressed conditions to elevated temperatures up to about 1000° F.

8. An alloy consisting essentially of about: 0.5 to 20% of the active eutectoid beta promoter copper, and containing at least one alpha promoter selected from the group consisting of aluminum, tin and antimony in total amount such that the sum of the aluminum plus one-third the tin plus one-third the antimony is less than 6% by weight of the total alloy, said alloy also containing about 1 to 20% of the alpha promoter zirconium, balance substantially titanium, characterized in being materially hardened and strengthened on heating above the critical temperature until a beta-containing microstructure is obtained, and thereupon rapidly cooling to a temperature substantially below the critical, said alloy being also

characterized by high stability after exposure in both stressed and unstressed conditions to elevated temperatures up to about 1000° F.

9. An alloy consisting essentially of about: 0.5 to 12% aluminum, 0.5 to 20% copper, balance substantially titanium, characterized in being forgeable and in being materially hardened and strengthened on heating above the critical temperature until a beta-containing microstructure is obtained and thereupon rapidly cooling to a temperature substantially below the critical.

10. An alloy consisting essentially of about: 4 to 8% aluminum, 2 to 4% copper, balance substantially titanium, characterized in having, as annealed, a tensile strength of at least 100,000 p. s. i., a minimum tensile elongation of about 2%, and in being materially hardened and strengthened on heating above the critical temperature until a beta-containing microstructure is obtained and thereupon rapidly cooling to a temperature substantially below the critical.

11. An alloy consisting essentially of about: 0.5 to under 6% aluminum, about 1 to 12% zirconium, about 0.5 to 20% copper, and the balance substantially titanium, characterized in having, as annealed, a tensile strength of at least 100,000 p. s. i., a minimum tensile elongation of about 2%, and in being materially hardened and strengthened on heating above the critical temperature until a beta-containing microstructure is obtained and thereupon rapidly cooling to a temperature substantially below the critical.

12. An alloy consisting essentially of about: 0.5 to 23% of at least one alpha promoter selected from the group consisting of aluminum, tin and antimony, about 1 to 20% of the alpha promoter zirconium, 0.5 to 20% of at least one active eutectoid beta promoter selected from the group consisting of copper, nickel, cobalt, silicon and beryllium, but not to exceed 12% of nickel and cobalt, 3% silicon and 2% beryllium, balance substantially titanium, characterized in having in the annealed condition a tensile strength of at least 100,000 p. s. i., a minimum tensile elongation of about 2%, and in being materially hardened and strengthened on heating above the critical temperature until a beta-containing microstructure is obtained and thereupon rapidly cooling to a temperature substantially below the critical.

13. An alloy consisting essentially of about: 8 to 14% tin, 5 to 8% copper, balance substantially titanium, characterized in being materially hardened and strengthened on heating above the critical temperature until a beta-containing microstructure is obtained and thereupon rapidly cooling to a temperature substantially below the critical.

14. An alloy consisting essentially of about: 0.5 to 23% of at least one element of the group aluminum, tin and antimony, but not to exceed 12% of aluminum and 19% antimony, 0.5 to 20% copper, balance titanium.

15. An alloy consisting of about: 0.5 to 23% of at least one element selected from the group consisting of aluminum, tin and antimony, but not to exceed 12% aluminum and 19% antimony, 0.5 to 12% of at least one element selected from the group consisting of nickel and cobalt, balance titanium.

16. An alloy consisting of about: 0.5 to 23% of at least one element selected from the group consisting of aluminum, tin and antimony, but not to exceed 12% aluminum and 19% antimony, 0.25 to 3% silicon and the balance titanium.

17. An alloy consisting of about: 0.5 to 23% of at least one element selected from the group consisting of aluminum, tin and antimony, but not to exceed 12% aluminum and 19% antimony, 0.1 to 2% beryllium, balance titanium.

18. The method of annealing an alloy according to claim 1 which comprises, heating above the beta transus until transformation to the beta phase is substantially complete, and thereupon slowly cooling at the rate of not

more than 5-10° F. per minute through the eutectoid temperature range.

19. The method of annealing an alloy according to claim 1 which comprises, heating at temperature of about 50-100° F. below the eutectoid temperature to remove strain and promote compound agglomeration and thereupon cooling substantially to room temperature.

20. The method of hardening an alloy according to claim 1 which comprises, heating above the eutectoid temperature until equilibrium of the alloy and transformation to the beta phase is substantially complete, and thereupon cooling rapidly through the eutectoid temperature at a rate sufficient to produce a fine eutectoid structure, said cooling being at least as rapid as an air cool.

21. The method of hardening an alloy according to claim 1 which comprises, heating the alloy above the beta transus until transformation to the beta phase is substantially complete, and thereupon cooling through the eutectoid temperature with sufficient rapidity to produce martensite, said cooling being at least as rapid as an air cool.

22. The method of hardening an alloy according to claim 1 which comprises, heating the alloy in the alpha-beta temperature range until equilibrium is established, and thereupon rapidly cooling through the eutectoid temperature, said cooling being at least as rapid as an air cool.

23. The method of hardening and tempering an alloy according to claim 1 which comprises, heating above the eutectoid temperature until equilibrium of the alloy and transformation to the beta phase is substantially complete, thereupon cooling at least as rapidly as an air cool

5

10

15

20

25

30

through the eutectoid temperature and at a rate sufficient to produce a fine eutectoid structure, and thereupon aging at temperature below the eutectoid temperature.

24. The method of hardening and tempering an alloy according to claim 1 which comprises, heating the alloy above the beta transus until transformation to the beta phase is substantially complete, thereupon cooling through the eutectoid temperature with sufficient rapidity to produce martensite, said cooling being at least as rapid as an air cool, and thereupon aging at temperature below the eutectoid temperature.

25. The method of hardening and tempering an alloy according to claim 1 which comprises, heating the alloy in the alpha-beta temperature range until equilibrium is established, thereupon rapidly cooling through the eutectoid temperature, said cooling being at least as rapid as an air cool, and thereupon aging at temperature below the eutectoid temperature.

26. The method of hardening an alloy according to claim 1 which comprises heating the alloy above the critical or eutectoid temperature and then cooling with sufficient rapidity to cause eutectoid decomposition of the beta formed on heating, said cooling being at least as rapid as an air cool, but slow enough to prevent undue distortion of the heat-treated alloy.

References Cited in the file of this patent

UNITED STATES PATENTS

|           |         |               |
|-----------|---------|---------------|
| 2,622,023 | Frazier | Dec. 16, 1952 |
| 2,669,513 | Jaffee  | Feb. 16, 1954 |

UNITED STATES PATENT OFFICE  
CERTIFICATE OF CORRECTION

Patent No. 2,867,534

January 6, 1959

Robert I. Jaffee et al.

It is hereby certified that error appears in the printed specification of the above numbered patent requiring correction and that the said Letters Patent should read as corrected below.

Column 9, Table IV, heading to second column, for "Est. Yield" read -- Est. Yield Strength --; same table, third column thereof, under the heading "Ultimate Strength", seventeenth item, for "1.2" read -- 122 --; column 14, Table XIII, under the heading "Composition (Wt. Percent), Bal. Titanium", first item, for "2Al-0 5Be" read -- 2Al-0.5Be --; second item, for "4Al-0 2Be" read -- 4Al-0.2Be --.

Signed and sealed this 14th day of April 1959.

(SEAL)  
Attest:

KARL H. AXLINE  
Attesting Officer

ROBERT C. WATSON  
Commissioner of Patents